



US007981837B2

(12) **United States Patent**  
**Shinohara et al.**

(10) **Patent No.:** **US 7,981,837 B2**  
(45) **Date of Patent:** **\*Jul. 19, 2011**

(54) **HEAT-SENSITIVE TRANSFER  
IMAGE-RECEIVING SHEET**

(75) Inventors: **Ryuji Shinohara**, Minami-ashigara (JP);  
**Hiroshi Takehara**, Minami-ashigara (JP); **Kiyoshi Irita**, Ashigarakami-gun (JP)

(73) Assignee: **Fujifilm Corporation**, Tokyo (JP)

(\*) Notice: Subject to any disclaimer, the term of this patent is extended or adjusted under 35 U.S.C. 154(b) by 950 days.

This patent is subject to a terminal disclaimer.

(21) Appl. No.: **11/819,842**

(22) Filed: **Jun. 29, 2007**

(65) **Prior Publication Data**

US 2008/0014382 A1 Jan. 17, 2008

(30) **Foreign Application Priority Data**

Jun. 30, 2006 (JP) ..... 2006-181224

(51) **Int. Cl.**

**B41M 5/035** (2006.01)  
**B41M 5/50** (2006.01)

(52) **U.S. Cl.** ..... **503/227; 428/32.39**

(58) **Field of Classification Search** ..... None  
See application file for complete search history.

(56)

**References Cited**

**U.S. PATENT DOCUMENTS**

|                |         |                   |
|----------------|---------|-------------------|
| 5,262,378 A    | 11/1993 | Kung et al.       |
| 7,223,513 B2   | 5/2007  | Nakane et al.     |
| 7,381,685 B2 * | 6/2008  | Oguma et al. .... |
| 7,485,402 B2 * | 2/2009  | Arai et al. ....  |

**FOREIGN PATENT DOCUMENTS**

|                |          |
|----------------|----------|
| JP 61-283595   | 12/1986  |
| JP 63-54975    | 3/1988   |
| JP 01-108090 A | 4/1989   |
| JP 02-070487 A | 3/1990   |
| JP 02-200489 A | 8/1990   |
| JP 5-209118    | 8/1993   |
| JP 06-171240 A | 6/1994   |
| JP 6-227160    | 8/1994   |
| JP 07-081249 A | 3/1995   |
| JP 2000-158831 | * 6/2000 |
| JP 2000-238440 | * 9/2000 |
| JP 2006-88691  | 4/2006   |

**OTHER PUBLICATIONS**

Japanese Office Action dated Feb. 8, 2011 for corresponding Japanese Patent Application No. 2007-082599.

\* cited by examiner

*Primary Examiner* — Bruce H Hess

(74) *Attorney, Agent, or Firm* — Sughrue Mion, PLLC

(57) **ABSTRACT**

A heat-sensitive transfer image-receiving sheet, containing; a support; at least one receptor layer containing a latex polymer, the latex polymer containing a repeating unit derived from vinyl chloride in a proportion of 50 mass % or above in the latex polymer; and at least one heat-insulation layer containing hollow latex polymer particles and a water-soluble polymer, the at least one heat-insulation layer being provided between the support and the at least one receptor layer.

**17 Claims, No Drawings**

## 1

HEAT-SENSITIVE TRANSFER  
IMAGE-RECEIVING SHEET

## FIELD OF THE INVENTION

The present invention relates to a heat-sensitive transfer image-receiving sheet.

## BACKGROUND OF THE INVENTION

Various heat transfer recording methods have been known so far. Among these methods, dye diffusion transfer recording systems attract attention as a process that can produce a color hard copy having an image quality closest to that of silver salt photography (see, for example, "Joho Kiroku (Hard Copy) to Sono Zairyō no Shintenkai (Information Recording (Hard Copy) and New Development of Recording Materials)", published by Toray Research Center Inc., 1993, pp. 241-285; and "Printer Zairyō no Kaihatsu (Development of Printer Materials)", published by CMC Publishing Co., Ltd., 1995, p. 180). Moreover, this system has advantages over silver salt photography: it is a dry system, it enables direct visualization from digital data, it makes reproduction simple, and the like.

In this dye diffusion transfer recording system, a heat-sensitive transfer sheet (hereinafter also referred to as an ink sheet) containing dyes is superposed on a heat-sensitive transfer image-receiving sheet (hereinafter also referred to as an image-receiving sheet), and then the ink sheet is heated by a thermal head whose exothermic action is controlled by electric signals, in order to transfer the dyes contained in the ink sheet to the image-receiving sheet, thereby recording an image information. Three colors: cyan, magenta, and yellow, are used for recording a color image by overlapping one color to other, thereby enabling transferring and recording a color image having continuous gradation for color densities.

In such a recording method in dye diffusion transfer system, it has been known that it is important 1) to make the image-receiving sheet have high heat insulation and cushion properties, and 2) to use a receiving layer high in affinity for dyes, in order to give a favorable image (see, for example, the above "Information Recording (Hard Copy) and New Development of Recording Materials", published by Toray Research Center Inc., 1993, pp. 241-285; and "Development of Printer Materials", published by CMC Publishing Co., Ltd., 1995, p. 180).

Thus, in some cases, a composite support in which a biaxial oriented (stretched) polyolefin film containing microvoids was laminated with a core layer made, for example, of paper, is used as a base material for the image-receiving sheet, to make the image-receiving sheet have heat insulation and cushion properties (see, for example, U.S. Pat. No. 866,282, and JP-A-3-268998 ("JP-A" means unexamined published Japanese patent application)). However, this method involves drawbacks of lowering the productivity and increasing the production cost, since, in that method, a receptor layer is to be formed by solvent coating after the lamination process.

As other known methods of making the image-receiving sheet show heat insulation and cushion properties, a method in which, for example, a foaming layer composed of a resin and a foaming agent (see, e.g., Japanese Patent No. 2541796) or a porous layer containing hollow polymer particles (see, e.g., JP-A-2006-82382), each layer having high cushion properties, is formed between the support and the receptor layer, is known. Since, according to these methods, it is possible to form a heat-insulating layer on a base material by coating, the methods have such advantage that it is possible to omit the lamination process that is necessitated by the afore-

## 2

mentioned method in which a composite support made of a biaxially-oriented polyolefin film containing microvoids is used.

In these techniques (Japanese Patent No. 2541796 and 5 JP-A-2006-82382), however, although the heat-insulating layers are formed by aqueous coating, the receptor layers are formed by solvent coating. As polymers usable in the receptor layers because of their high affinity for dyes, polyester resins, vinyl chloride resins, and polycarbonate resins are known 10 (see, e.g., JP-A-61-283595, JP-A-5-209118 and JP-A-6-227160). While solvent coating is adopted in many of the methods for forming those receptor layers, no method using a latex polymer permitting aqueous coating is carried out yet. Accordingly, the heat-sensitive transfer image-receiving 15 sheet production inevitably entails a sequential coating process that first comes the formation of a heat-insulating layer by aqueous coating, and then the formation of a receptor layer by solvent coating, so it is hard to say that the methods as mentioned above are sufficient from the viewpoint of productivity.

In the silver-salt photographic industry, on the other hand, it is known that productivity is largely enhanced by adopting a simultaneous aqueous multilayer coating method in forming on a support a plurality of layers differing in their functions (JP-A-63-54975; and by Edgar B. Gutoff et al., "Coating and Drying Defects: Troubleshooting Operating Problems", pages 101-103, John Wiley & Sons (1995)). Further, in the field of heat-sensitive transfer image-receiving sheets also, simultaneous multilayer coating has recently 20 been put forth (JP-A-2006-88691). The aqueous multilayer coating has greater advantages than the solvent coating, in not only productivity, but also prevention of air pollution and hazard of fire, and improvement in working hygiene, but it has many problems to settle. Moreover, it is demanded for heat-sensitive transfer image-receiving sheets that they have much 25 higher dyeing property than before, give sufficiently high sensitivity and maximum density, and exhibit good releasing property from ink sheets (no adhesion remains between those two sheets).

## 40 SUMMARY OF THE INVENTION

The present invention resides in a heat-sensitive transfer image-receiving sheet, which comprises;

45 a support;  
at least one receptor layer containing a latex polymer, said latex polymer containing a repeating unit derived from vinyl chloride in a proportion of 50 mass % or above in the latex polymer; and  
50 at least one heat-insulation layer containing hollow latex polymer particles and a water-soluble polymer, said at least one heat-insulation layer being provided between the support and the at least one receptor layer.

Other and further features and advantages of the invention

55 will appear more fully from the following description.

## DETAILED DESCRIPTION OF THE INVENTION

According to the present invention, there is provided the 60 following means:

(1) A heat-sensitive transfer image-receiving sheet, comprising;  
a support;  
at least one receptor layer containing a latex polymer, said 65 latex polymer containing a repeating unit derived from vinyl chloride in a proportion of 50 mass % or above in the latex polymer; and

at least one heat-insulation layer containing hollow latex polymer particles and a water-soluble polymer, said at least one heat-insulation layer being provided between the support and the at least one receptor layer;

(2) The heat-sensitive transfer image-receiving sheet according to Item (1), wherein the latex polymer contained in the at least one receptor layer is a copolymer of vinyl chloride and an acrylic acid ester;

(3) The heat-sensitive transfer image-receiving sheet according to Item (2), wherein the latex polymer contained in the at least one receptor layer is a copolymer of vinyl chloride and at least two acrylic acid esters;

(4) The heat-sensitive transfer image-receiving sheet according to Item (2) or (3), wherein the number of carbon atoms in an alcohol-derived moiety of the acrylic acid ester is 1 to 8;

(5) The heat-sensitive transfer image-receiving sheet according to any of Items (2) to (4), wherein the number of carbon atoms in an alcohol-derived moiety of the acrylic acid ester is 1, and wherein a repeating unit derived from said acrylic acid ester is contained in the copolymer in a proportion of 10 to 45 mass %;

(6) The heat-sensitive transfer image-receiving sheet according to any of Items (2) to (4), wherein the number of carbon atoms in an alcohol-derived moiety of the acrylic acid ester is 2, and wherein a repeating unit derived from said acrylic acid ester is contained in the copolymer in a proportion of 5 to 45 mass %;

(7) The heat-sensitive transfer image-receiving sheet according to any of Items (2) to (4), wherein the number of carbon atoms in an alcohol-derived moiety of the acrylic acid ester is 3, and wherein a repeating unit derived from said acrylic acid ester is contained in the copolymer in a proportion of 5 to 35 mass %;

(8) The heat-sensitive transfer image-receiving sheet according to any of Items (2) to (4), wherein the number of carbon atoms in an alcohol-derived moiety of the acrylic acid ester is 4, and wherein a repeating unit derived from said acrylic acid ester is contained in the copolymer in a proportion of 4 to 30 mass %;

(9) The heat-sensitive transfer image-receiving sheet according to any of Items (2) to (4), wherein the number of carbon atoms in an alcohol-derived moiety of the acrylic acid ester is 6, and wherein a repeating unit derived from said acrylic acid ester is contained in the copolymer in a proportion of 3 to 28 mass %;

(10) The heat-sensitive transfer image-receiving sheet according to any of Items (2) to (4), wherein the number of carbon atoms in an alcohol-derived moiety of each acrylic acid ester is 8, and wherein a repeating unit derived from said acrylic acid ester is contained in the copolymer in a proportion of 2 to 25 mass %;

(11) The heat-sensitive transfer image-receiving sheet according to any of Items (1) to (10), wherein the latex polymer contained in the at least one receptor layer is a copolymer of vinyl chloride and vinyl acetate;

(12) The heat-sensitive transfer image-receiving sheet according to Item (11), wherein a repeating unit derived from the vinyl acetate is contained in the copolymer in a proportion of 3 to 30 mass %;

(13) The heat-sensitive transfer image-receiving sheet according to Item (1), wherein the latex polymer contained in the at least one receptor layer is a copolymer of vinyl chloride, at least one acrylic acid ester, and vinyl acetate; and

(14) The heat-sensitive transfer image-receiving sheet according to any of Items (1) to (13), which is produced

through simultaneous coating of the at least one receptor layer and the at least one heat-insulating layer.

The present invention is explained in detail below.

First, the heat-sensitive transfer image-receiving sheet (image-receiving sheet) of the present invention is explained.

The heat-sensitive transfer image-receiving sheet of the present invention is provided with at least one dye-receiving layer (receptor layer) and at least one heat insulation layer on a support. It is preferable to form an undercoat layer between the receptor layer and the support. As the undercoat layer, for example, a white background control layer, a charge control layer, an adhesive layer, and a primer layer can be formed. Also, the heat insulation layer is preferably formed between the undercoat layer and the support. It is preferable that a curling control layer, a writing layer, or a charge-control layer be formed on the backside of the support. Each of these layers is applied, using a usual method, such as a roll coating, a bar coating, a gravure coating, a gravure reverse coating, a dye coating, a slide coating, and a curtain coating. In practicing the present invention, a method capable of conducting a simultaneous multi-layer coating, such as the slide coating and the curtain coating, is preferable.

(Receptor Layer)

The receptor layer performs functions of receiving dyes to be transferred from an ink sheet and retaining images thus formed. The image-receiving sheet of the present invention has at least one receptor layer preferably containing at least one thermoplastic receiving polymer that can receive a dye.

The receiving polymer is preferably used, as it is dispersed in a water-soluble dispersion medium as a latex polymer. In addition, the receptor layer preferably contains a water-soluble polymer together with the latex polymer. Co-presence of the latex polymer and the water-soluble polymer allows presence of the water-soluble polymer, which is hardly dyable, among the latex polymers and prevents diffusion of the dye fixed on the latex polymer, and consequently, reduces changes in the color sharpness of the receptor layer with the lapse of time and forms a recorded image smaller in changes for its transferred image quality with the lapse of time.

The receptor layer may contain, in addition to the latex polymer of the receiving polymer, another latex polymer having a different function, for example, for the purpose of adjusting the elastic modulus of the film.

<Latex Polymer>

The latex polymer used in the present invention is explained.

Generally, latex polymers are described in "Gosei Jushi Emulsion (Synthetic Resin Emulsion)", compiled by Taira Okuda and Hiroshi Inagaki, issued by Kobunshi Kankai Kai (1978); "Gosei Latex no Oyo (Application of Synthetic Latex)", compiled by Takaaki Sugimura, Yasuo Kataoka, Souichi Suzuki, and Keishi Kasahara, issued by Kobunshi Kankai Kai (1993); Soichi Muroi, "Gosei Latex no Kagaku (Chemistry of Synthetic Latex)", issued by Kobunshi Kankai Kai (1970); Yoshiaki Miyosawa (supervisor) "Suisei Coating-Zairyo no Kaihatsu to Oyo (Development and Application of Aqueous Coating Material)", issued by CMC Publishing Co., Ltd. (2004); JP-A-64-538, and so forth.

In the heat-sensitive transfer image-receiving sheet of the present invention, the latex polymer used in the receptor layer is a dispersion in which a water-insoluble hydrophobic polymer(s) is dispersed as fine particles in a water-soluble dispersion medium. Multiple kinds of different latex polymers may be used in combination as the latex polymer, but the latex polymer for use in the present invention preferably contains at least vinyl chloride as a monomer unit, i.e., contains a repeating unit derived from vinyl chloride, and the vinyl chloride

unit constitutes preferably at least 50 mass %, more preferably at least 65 mass %, further preferably 70 to 95 mass %, of the total polymers in the receptor layer.

In synthesis of the latex polymer containing a monomer unit, i.e. a repeating unit, derived from vinyl chloride that can be used in the present invention, no particular limitation is imposed on another monomer that can be used in combination with the aforementioned vinyl chloride monomer, and any of the following monomer groups (a) to (j) may be preferably used as one polymerizable in a usual radical polymerization or ion polymerization method. Those monomers may be selected singly or combined freely, to synthesize the latex polymer.

—Monomer Groups (a) to (j)—

(a) Conjugated dienes: 1,3-pentadiene, isoprene, 1-phenyl-1,3-butadiene, 1- $\alpha$ -naphthyl-1,3-butadiene, 1- $\beta$ -naphthyl-1,3-butadiene, cyclopentadiene, etc.

(b) Olefins: ethylene, propylene, vinyl chloride, vinylidene chloride, 6-hydroxy-1-hexene, 4-pentenoic acid, methyl 8-nonenate, vinylsulfonic acid, trimethylvinylsilane, trimethoxyvinylsilane, 1,4-divinylcyclohexane, 1,2,5-trivinylcyclohexane, etc.

(c)  $\alpha,\beta$ -unsaturated carboxylates: alkyl acrylates, such as methyl acrylate, ethyl acrylate, butyl acrylate, cyclohexyl acrylate, 2-ethylhexyl acrylate, and dodecyl acrylate; substituted alkyl acrylates, such as 2-chloroethyl acrylate, benzyl acrylate, and 2-cyanoethyl acrylate; alkyl methacrylates, such as methyl methacrylate, butyl methacrylate, 2-ethylhexyl methacrylate, and dodecyl methacrylate; substituted alkyl methacrylates, such as 2-hydroxyethyl methacrylate, glycidyl methacrylate, glycerin monomethacrylate, 2-acetoxyethyl methacrylate, tetrahydrofurfuryl methacrylate, 2-methoxyethyl methacrylate, polypropylene glycol monomethacrylates (mole number of added polyoxypropylene=2 to 100), 3-N,N-dimethylaminopropyl methacrylate, chloro-3-N,N,N-trimethylammoniopropyl methacrylate, 2-carboxyethyl methacrylate, 3-sulfopropyl methacrylate, 4-oxy sulfobutyl methacrylate, 3-trimethoxysilylpropyl methacrylate, allyl methacrylate, and 2-isocyanatoethyl methacrylate; derivatives of unsaturated dicarboxylic acids, such as monobutyl maleate, dimethyl maleate, monomethyl itaconate, and dibutyl itaconate; multifunctional esters, such as ethylene glycol diacrylate, ethylene glycol dimethacrylate, 1,4-cyclohexane diacrylate, pentaerythritol tetramethacrylate, pentaerythritol triacrylate, trimethylolpropane triacrylate, trimethylolethane triacrylate, dipentaerythritol pentamethacrylate, pentaerythritol hexaacrylate, and 1,2,4-cyclohexane tetramethacrylate; etc. Of these, an acrylic acid ester and a methacrylic acid ester are preferred.

(d)  $\alpha,\beta$ -unsaturated carboxylic amides: e.g. acrylamide, methacrylamide, N-methylacrylamide, N,N-dimethylacrylamide, N-methyl-N-hydroxyethylmethacrylamide, N-tert-butylacrylamide, N-tert-octylmethacrylamide, N-cyclohexylacrylamide, N-phenylacrylamide, N-(2-acetoacetoxyethyl)acrylamide, N-acryloylmorpholine, diacetone acrylamide, itaconic diamide, N-methylmaleimide, 2-acrylamide-methylpropane sulfonic acid, methylenebisacrylamide, dimethacryloylpiperazine, etc.

(e) Unsaturated nitriles: acrylonitrile, methacrylonitrile, etc.

(f) Styrene and derivatives thereof: styrene, vinyltoluene, p-tert-butylstyrene, vinylbenzoic acid, methyl vinylbenzoate,  $\alpha$ -methylstyrene, p-chloromethylstyrene, vinyl-naphthalene, p-hydroxymethylstyrene, sodium p-styrene-sulfonate, potassium p-styrenesulfonate, p-amino-methylstyrene, 1,4-divinylbenzene, etc.

(g) Vinyl ethers: methyl vinyl ether, butyl vinyl ether, methoxyethyl vinyl ether, etc.

(h) Vinyl esters: vinyl acetate, vinyl propionate, vinyl benzoate, vinyl salicylate, vinyl chloroacetate, etc.

5 (i)  $\alpha,\beta$ -unsaturated carboxylic acids and salts thereof: acrylic acid, methacrylic acid, itaconic acid, maleic acid, sodium acrylate, ammonium methacrylate, potassium itaconate, etc.

10 (j) Other polymerizable monomers: N-vinylimidazole, 4-vinylpyridine, N-vinylpyrrolidone, 2-vinylloxazoline, 2-isopropenylloxazoline, divinylsulfone, etc.

In a preferred aspect of the latex polymer containing a repeating unit derived from vinyl chloride, which is used in the receptor layer according to the present invention, a 15 copolymer containing vinyl chloride as a monomer unit can be used. The monomer(s) to be copolymerized with the vinyl chloride monomer is preferably (b), (c), (e), (g), (i) or (h), more preferably (c) or (h), of the above-mentioned ones. Of these monomers, acrylic acid esters and vinyl esters are preferred, acrylic acid esters having 1 to 8 carbon atoms in their 20 respective alcohol-derived moieties and vinyl acetate are more preferred, and acrylic acid esters having 1 to 8 carbon atoms in their respective alcohol-derived moieties are especially preferred.

25 The monomers to be copolymerizable with the foregoing vinyl chloride monomer may be used singly or as combinations of two or more thereof. Preferable examples of such a copolymer include a vinyl chloride/vinyl acetate copolymer, a vinyl chloride/acrylic acid ester copolymer; a vinyl chloride/acrylic acid ester/acrylic acid ester, in which the latter is 30 different from the former, terpolymer; and a vinyl chloride/vinyl acetate/acrylic acid ester terpolymer. Of these copolymers, a vinyl chloride/acrylic acid ester copolymer is more preferred to other ones. In those cases, the proportion of vinyl 35 chloride repeating unit (monomer) is preferably from 50% to 98%.

As to the latex of vinyl chloride/acrylic acid ester copolymer used in the present invention, the number of carbon atoms in alcohol-derived moiety of the acrylic acid ester is not 40 particularly limited, but it is preferably 1 to 8, more preferably 1, 2, 3, 4, 6 or 8, further preferably 2, 3 or 4, most preferably 2 or 4.

45 In view of dye transferability at the time of image formation, adhesiveness to ink sheets, and easiness of handling during the coating operation, the latex of the vinyl chloride/acrylic acid ester copolymer is chosen as appropriate. Those properties are generally dependent on what glass transition temperature (Tg) the chosen latex has. For instance, the lower Tg a latex copolymer has, the latex copolymer generally 50 becomes more favorable for transferability of dyes; and the higher Tg a copolymer latex has, the copolymer latex becomes more favorable in point of poor adhesion to ink ribbons. With respect to the easiness of handling during the coating operation, it is known that the higher Tg a copolymer 55 latex has, the more favorably the copolymer latex can be used because coating burrs are hard to occur.

Under these circumstances, we found that a vinyl chloride/acrylic acid ester copolymer in which the number of carbon atoms contained in the alcohol-derived moiety is 4, can be 60 preferably used, because of its superiority in transferability to other vinyl chloride/acrylic acid ester copolymers having the same level of Tg, thereby achieving a preferable embodiment of the present invention.

Furthermore, we also found that, when image-receiving 65 sheets for use in sublimation printers are formed using coating techniques, a vinyl chloride/acrylic acid ester copolymer in which the number of carbon atoms contained in the alco-

hol-derived moiety is 2, can provide the sheets with more favorable surface conditions than other vinyl chloride/acrylic acid ester copolymers having the same level of  $T_g$ , thereby achieving another preferable embodiment of the present invention.

In the latex of a vinyl chloride/acrylic acid ester copolymer, the proportion of acrylic acid ester repeating unit is preferably from 10 mass % to 45 mass %, more preferably from 15 mass % to 40 mass %, most preferably from 20 mass % to 35 mass %, when the number of carbon atoms in the alcohol-derived moiety of acrylic acid ester repeating unit is 1.

The proportion of acrylic acid ester repeating unit is preferably from 5 mass % to 45 mass %, more preferably from 10 mass % to 40 mass %, most preferably from 20 mass % to 30 mass %, when the number of carbon atoms in the alcohol-derived moiety of acrylic acid ester repeating unit is 2.

The proportion of acrylic acid ester repeating unit is preferably from 5 mass % to 35 mass %, more preferably from 10 mass % to 30 mass %, most preferably from 15 mass % to 25 mass %, when the number of carbon atoms in the alcohol-derived moiety of acrylic acid ester repeating unit is 3.

The proportion of acrylic acid ester repeating unit is preferably from 4 mass % to 30 mass %, more preferably from 5 mass % to 25 mass %, most preferably from 8 mass % to 20 mass %, when the number of carbon atoms in the alcohol-derived moiety of acrylic acid ester repeating unit is 4.

The proportion of acrylic acid ester repeating unit is preferably from 3 mass % to 28 mass %, more preferably from 5 mass % to 25 mass %, most preferably from 7 mass % to 20 mass %, when the number of carbon atoms in the alcohol-derived moiety of acrylic acid ester repeating unit is 6.

The proportion of acrylic acid ester repeating unit is preferably from 2 mass % to 25 mass %, more preferably from 4 mass % to 25 mass %, most preferably from 6 mass % to 20 mass %, when the number of carbon atoms in the alcohol-derived moiety of acrylic acid ester repeating unit is 8.

In the latex of a vinyl chloride/vinyl acetate copolymer, the proportion of vinyl acetate repeating unit is preferably from 3 mass % to 30 mass %, more preferably from 5 mass % to 25 mass %, most preferably from 8 mass % to 20 mass %.

In a latex of a vinyl chloride/acrylic acid ester/acrylic acid ester (which is different from the former) terpolymer, the total proportion of these two types of acrylic acid ester repeating units is preferably from 2 mass % to 45 mass %.

In a latex of a vinyl chloride/vinyl acetate/acrylic acid ester terpolymer, the total proportion of vinyl acetate and acrylic acid ester repeating units is preferably from 2 mass % to 45 mass %.

These polymers may be straight-chain, branched, or cross-linked polymers. In the case of the copolymers, these copolymers may be either random copolymers or block copolymers. The molecular weight of each of these polymers is preferably 5,000 to 1,000,000, and further preferably 10,000 to 500,000 in terms of number average molecular weight. Polymers having excessively small molecular weight impart insufficient dynamic strength to the layer containing the latex, and polymers having excessively large molecular weight bring about poor filming ability, and therefore both cases are not preferable. Crosslinkable latex polymers are also preferably used.

The average diameter of the dispersed particles is preferably in the range of approximately 1 to 50,000 nm, more preferably 5 to 1,000 nm. The particle diameter distribution of the dispersed particles is not particularly limited, and thus, the particles may have a wide particle diameter distribution or a monodispersion-like particle diameter distribution. The average particle diameter of such an order can be measured, for

example, with SUB-MICRON PARTICLE ANALYZER (Model N4SD, trade name, manufactured by Coulter).

The latex polymer having a different structure, which can be used in combination with the latex polymer containing a monomer unit derived from vinyl chloride, is not particularly limited. As the aforementioned latex polymer of different structure, use may be preferably made of hydrophobic polymers, such as acrylic-series polymers, polyesters, rubbers (e.g., SBR resins), polyurethanes, polyvinyl chlorides, polyvinyl acetates, polyvinylidene chlorides, and polyolefins. These polymers may be straight-chain, branched, or cross-linked polymers, and may be the so-called homopolymers obtained by polymerizing single type of monomers, or copolymers obtained by polymerizing two or more types of monomers. In the case of the copolymers, these copolymers may be either random copolymers or block copolymers. The molecular weight of each of these polymers is preferably 5,000 to 1,000,000, and further preferably 10,000 to 500,000 in terms of number average molecular weight. A polymer having an excessively small molecular weight imparts insufficient dynamic strength to a layer containing a latex of the polymer, and a polymer having an excessively large molecular weight brings about poor filming ability, and therefore both cases are not preferable. Crosslinkable latex polymers are also preferably used.

The latex polymer for use in the present invention may be latex of the so-called core/shell type, other than ordinary latex polymer of a uniform structure. When using a core/shell type latex polymer, it is preferred in some cases that the core and the shell have different glass transition temperatures. The glass transition temperature ( $T_g$ ) of the latex polymer for use in the present invention is preferably  $-30^{\circ}\text{C}$ . to  $100^{\circ}\text{C}$ ., more preferably  $0^{\circ}\text{C}$ . to  $80^{\circ}\text{C}$ ., further more preferably  $10^{\circ}\text{C}$ . to  $70^{\circ}\text{C}$ ., and especially preferably  $15^{\circ}\text{C}$ . to  $60^{\circ}\text{C}$ .

The glass transition temperature ( $T_g$ ) can be calculated, according to the following equation:

$$1/T_g = \Sigma(X_i/T_{gi})$$

wherein, assuming that the polymer is a copolymer composed of  $n$  monomers from  $i=1$  to  $i=n$ ,  $X_i$  is a weight fraction of the  $i$ -th monomer unit ( $\Sigma X_i = 1$ ) and  $T_{gi}$  is glass transition temperature (measured in absolute temperature) of a homopolymer formed from the  $i$ -th monomer. The symbol  $\Sigma$  means the sum of  $i=1$  to  $i=n$ . The value of the glass transition temperature of a homopolymer formed from each monomer ( $T_{gi}$ ) can be adopted from those by J. Brandrup and E. H. Immergut, "Polymer Handbook, 3rd. Edition", Wiley-Interscience (1989).

The glass transition temperature ( $T_g$ ) of the latex polymer having a different structure that can be used in combination with the latex polymer according to the present invention containing vinyl chloride as a monomer unit, is preferably in the range of  $-30^{\circ}\text{C}$ . to  $100^{\circ}\text{C}$ ., more preferably  $0^{\circ}\text{C}$ . to  $80^{\circ}\text{C}$ ., still more preferably  $20^{\circ}\text{C}$ . to  $70^{\circ}\text{C}$ ., from the viewpoints of brittleness for working (film-forming properties) and image preservability. A blend of two or more types of polymers can be used as the binder. When a blend of two or more polymers is used, the average  $T_g$  obtained by summing up the  $T_g$  of each polymer weighted by its proportion, is preferably within the foregoing range. Also, when phase separation occurs or when a core-shell structure is adopted, the weighted average  $T_g$  is preferably within the foregoing range.

The latex polymer for use in the present invention preferably has a minimum film-forming temperature (MFT) of from  $-30$  to  $90^{\circ}\text{C}$ ., more preferably from  $0$  to  $70^{\circ}\text{C}$ . In order to control the minimum film-forming temperature, a film-forming aid may be added. The film-forming aid is also called

a temporary plasticizer, and it is an organic compound (usually an organic solvent) that lowers the minimum film-forming temperature of a latex polymer. It is described, for example, by Souichi Muroi, "Gosei Latex no Kagaku (Chemistry of Synthetic Latex)", issued by Kobunshi Kanko Kai (1970). Preferable examples of the film-forming aid are listed below, but the compounds that can be used in the present invention are not limited to the following specific examples.

Z-1: Benzyl alcohol

Z-2: 2,2,4-Trimethylpentanediol-1,3-monoisobutyrate

Z-3: 2-Dimethylaminoethanol

Z-4: Diethylene glycol

The latex polymer containing a repeating unit derived from vinyl chloride that can be used in the present invention, is commercially available, and polymers described below may be utilized. Examples thereof include G351 and G576 (trade names, manufactured by Nippon Zeon Co., Ltd.); VINYBLAN 240, 270, 277, 375, 386, 609, 550, 601, 602, 630, 660, 671, 683, 680, 680S, 681N, 685R, 277, 380, 381, 410, 430, 432, 860, 863, 865, 867, 900, 900GT, 938 and 950 (trade names, manufactured by Nissin Chemical Industry Co., Ltd.).

Latex polymers having a different structure that can be used in combination with the latex polymer containing a repeating unit derived from vinyl chloride, are also commercially available, and polymers described below may be utilized. Examples of the acrylic-series polymers include Cevian A-4635, 4718, and 4601 (trade names, manufactured by Daicel Chemical Industries); Nipol Lx811, 814, 821, 820, 855 (P-17: Tg 36° C.), and 857×2 (P-18: Tg 43° C.) (trade names, manufactured by Nippon Zeon Co., Ltd.); Voncoat R3370 (P-19: Tg 25° C.), and 4280 (P-20: Tg 15° C.) (trade names, manufactured by Dai-Nippon Ink & Chemicals, Inc.); Julimer ET-410 (P-21: Tg 44° C.) (trade name, manufactured by Nihon Junyaku K.K.); AE116 (P-22: Tg 50° C.), AE119 (P-23: Tg 55° C.), AE121 (P-24: Tg 58° C.), AE125 (P-25: Tg 60° C.), AE134 (P-26: Tg 48° C.), AE137 (P-27: Tg 48° C.), AE140 (P-28: Tg 53° C.), and AE173 (P-29: Tg 60° C.) (trade names, manufactured by JSR Corporation); Aron A-104 (P-30: Tg 45° C.) (trade name, manufactured by Toagosei Co., Ltd.); NS-600X, and NS-620X (trade names, manufactured by Takamatsu Yushi K.K.); VINYBLAN 2580, 2583, 2641, 2770, 2770H, 2635, 2886, 5202C, and 2706 (trade names, manufactured by Nissin Chemical Industry Co., Ltd.).

Examples of the polyesters include FINETEX ES650, 611, 675, and 850 (trade names, manufactured by Dainippon Ink and Chemicals, Incorporated); WD-size, and WMS (trade names, manufactured by Eastman Chemical Ltd.); A-110, A-115GE, A-120, A-121, A-124GP, A-124S, A-160P, A-210, A-215GE, A-510, A-513E, A-515GE, A-520, A-610, A-613, A-615GE, A-620, WAC-10, WAC-15, WAC-17XC, WAC-20, S-110, S-110EA, S-111SL, S-120, S-140, S-140A, S-250, S-252G, S-250S, S-320, S-680, DNS-63P, NS-122L, NS-122LX, NS-244LX, NS-140L, NS-141 LX, and NS-282LX (trade names, manufactured by Takamatsu Yushi K.K.); Aronmelt PES-1000 series, and PES-2000 series (trade names, manufactured by Toagosei Co., Ltd.); Bironal MD-1100, MD-1200, MD-1220, MD-1245, MD-1250, MD-1335, MD-1400, MD-1480, MD-1500, MD-1930, and MD-1985 (trade names, manufactured by Toyobo Co., Ltd.); and Ceporjon ES (trade name, manufactured by Sumitomo Seika Chemicals Co., Ltd.).

Examples of the polyurethanes include HYDRAN AP10, AP20, AP30, AP40, and 101H, Vondic 1320NS and 1610NS (trade names, manufactured by Dainippon Ink and Chemicals, Incorporated); D-1000, D-2000, D-6000, D-4000, and D-9000 (trade names, manufactured by Dainichi Seika Color & Chemicals Mfg. Co., Ltd.); NS-155X, NS-310A,

NS-310X, and NS-311X (trade names, manufactured by Takamatsu Yushi K.K.); Elastron (trade name, manufactured by Dai-ichi Kogyo Seiyaku Co., Ltd.).

Examples of the rubbers include LACSTAR 7310K, 3307B, 4700H, and 7132C (trade names, manufactured by Dainippon Ink & Chemicals Incorporated); Nipol Lx416, LX410, LX430, LX435, LX110, LX415A, LX438C, 2507H, LX303A, LX407BP series, V1004, and MH5055 (trade names, manufactured by Nippon Zeon Co., Ltd.).

10 Examples of the polyolefins include Chemipearl S120, SA100, and V300 (P-40: Tg 80° C.) (trade names, manufactured by Mitsui Petrochemical); Voncoat 2830, 2210, and 2960 (trade names, manufactured by Dainippon Ink and Chemicals, Incorporated); Zaikusen and Ceporjon G (trade names, manufactured by Sumitomo Seika Chemicals Co., Ltd.). Examples of the copolymer nylons include Ceporjon PA (trade name, manufactured by Sumitomo Seika Chemicals Co., Ltd.).

15 Examples of the polyvinyl acetates include VINYBLAN 1080, 1082, 1085W, 1108W, 1108S, 1563M, 1566, 1570, 1588C, A22J7-F2, 1128C, 1137, 1138, A20J2, A23J1, A23J1, A23K1, A23P2E, A68J1N, 1086A, 1086, 1086D, 1108S, 1187, 1241LT, 1580N, 1083, 1571, 1572, 1581, 4465, 4466, 4468W, 4468S, 4470, 4485LL, 4495LL, 1023, 1042, 1060, 25 1060S, 1080M, 1084W, 1084S, 1096, 1570K, 1050, 1050S, 3290, 1017AD, 1002, 1006, 1008, 1107L, 1225, 1245L, GV-6170, GV-6181, 4468W, and 4468S (trade names, manufactured by Nissin Chemical Industry Co., Ltd.).

20 These latex polymers may be used singly, or two or more of these polymers may be blended, if necessary.

In the receptor layer for use in the present invention, a ratio of the latex polymer containing a vinyl chloride monomer unit is preferably 50 mass % or more of the whole solid content in the layer.

25 The dispersed state may be one in which polymer is emulsified in a dispersion medium, one in which polymer is underwent emulsion polymerization, one in which polymer is underwent micelle dispersion, one in which polymer molecules partially have a hydrophilic structure and thus the 30 molecular chains themselves are dispersed in a molecular state, or the like.

The latex polymer for use in the present invention can be easily obtained by a solution polymerization method, a suspension polymerization method, an emulsion polymerization method, a dispersion polymerization method, an anionic polymerization method, a cationic polymerization method, or the like. Above all, an emulsion polymerization method in which the polymer is obtained as a latex is the most preferable. Also, a method is preferable in which the polymer is prepared in a solution, and the solution is neutralized, or an emulsifier is added to the solution, to which water is then added, to prepare an aqueous dispersion by forced stirring. For example, an emulsion polymerization method comprises conducting polymerization under stirring at about 30° C. to 55 about 100° C. (preferably 60° C. to 90° C.) for 3 to 24 hours, by using water or a mixed solvent of water and a water-miscible organic solvent (such as methanol, ethanol, or acetone) as a dispersion medium, a monomer mixture in an amount of 5 mass % to 150 mass % based on the amount of the dispersion medium, an emulsifier and a polymerization initiator. Various conditions, such as the dispersion medium, the monomer concentration, the amount of initiator, the amount of emulsifier, the amount of dispersant, the reaction temperature, and the method for adding monomers, are suitably determined considering the type of the monomers to be used. Furthermore, it is preferable to use a dispersant when necessary.

## 11

Generally, the emulsion polymerization method can be conducted according to the disclosures of the following documents: "Gosei Jushi Emulsion (Synthetic Resin Emulsions)" (edited by Taira Okuda and Hiroshi Inagaki and published by Kobunshi Kankokai (1978)); "Gosei Latex no Oyo (Applications of Synthetic Latexes)" (edited by Takaaki Sugimura, Yasuo Kataoka, Soichi Suzuki, and Keiji Kasahara and published by Kobunshi Kankokai (1993)); and "Gosei Latex no Kagaku (Chemistry of Synthetic Latexes)" (edited by Soichi Muroi and published by Kobunshi Kankokai (1970)). The emulsion polymerization method for synthesizing the latex polymer for use in the present invention may be a batch polymerization method, a monomer (continuous or divided) addition method, an emulsion addition method, or a seed polymerization method. The emulsion polymerization method is preferably a batch polymerization method, a monomer (continuous or divided) addition method, or an emulsion addition method in view of the productivity of latex.

The polymerization initiator may be any polymerization initiator having radical generating ability. The polymerization initiator to be used may be selected from inorganic peroxides, such as persulfates and hydrogen peroxide; peroxides described in the organic peroxide catalogue of NOF Corporation; and azo compounds as described in the azo polymerization initiator catalogue of Wako Pure Chemical Industries, Ltd. Among them, water-soluble peroxides, such as persulfates, and water-soluble azo compounds, as described in the azo polymerization initiator catalogue of Wako Pure Chemical Industries, Ltd., are preferable; ammonium persulfate, sodium persulfate, potassium persulfate, azobis(2-methyl-propionamidine) hydrochloride, azobis(2-methyl-N-(2-hydroxyethyl)propionamide), and azobiscyanovaleric acid are more preferable; and peroxides, such as ammonium persulfate, sodium persulfate, and potassium persulfate, are especially preferable, from the viewpoints of image preservability, solubility, and cost.

The amount of the polymerization initiator to be added is, based on the total amount of monomers, preferably 0.3 mass % to 2.0 mass %, more preferably 0.4 mass % to 1.75 mass %, and especially preferably 0.5 mass % to 1.5 mass %.

The polymerization emulsifier to be used may be selected from anionic surfactants, nonionic surfactants, cationic surfactants, and ampholytic surfactants. Among them, anionic surfactants are preferable from the viewpoints of dispersibility and image preservability. Sulfonic acid type anionic surfactants are more preferable because polymerization stability can be ensured even with a small addition amount and they have resistance to hydrolysis. Long chain alkyl diphenyl ether disulfonic acid salts (whose typical example is PELEX SS-H (trade name) manufactured by Kao Corporation,) are still more preferable, and low electrolyte types, such as PIONIN A-43-S (trade name, manufactured by Takemoto Oil & Fat Co., Ltd.) are especially preferable.

The amount of sulfonic acid type anionic surfactant as the polymerization emulsifier is preferably 0.1 mass % to 10.0 mass %, more preferably 0.2 mass % to 7.5 mass %, and especially preferably 0.3 mass % to 5.0 mass %, based on the total amount of monomers.

It is preferable to use a chelating agent in synthesizing the latex polymer to be used in the present invention. The chelating agent is a compound capable of coordinating (chelating) a polyvalent ion, such as metal ion (e.g., iron ion) or alkaline earth metal ion (e.g., calcium ion), and examples of the chelate compound which can be used include the compounds described in JP-B-6-8956 ("JP-B" means examined Japanese patent publication), U.S. Pat. No. 5,053,322, JP-A-4-73645, JP-A-4-127145, JP-A-4-247073, JP-A-4-305572, JP-A-6-

## 12

11805, JP-A-5-173312, JP-A-5-66527, JP-A-5-158195, JP-A-6-118580, JP-A-6-110168, JP-A-6-161054, JP-A-6-175299, JP-A-6-214352, JP-A-7-114161, JP-A-7-114154, JP-A-7-120894, JP-A-7-199433, JP-A-7-306504, JP-A-9-43792, JP-A-8-314090, JP-A-10-182571, JP-A-10-182570, and JP-A-11-190892.

Preferred examples of the chelating agent include inorganic chelate compounds (e.g., sodium tripolyphosphate, sodium hexametaphosphate, sodium tetrapolyphosphate), 10 aminopolycarboxylic acid-based chelate compounds (e.g., nitrilotriacetic acid, ethylenediaminetetraacetic acid), organic phosphonic acid-based chelate compounds (e.g., compounds described, for example, in Research Disclosure No. 18170, JP-A-52-102726, JP-A-53-42730, JP-A-56-97347, JP-A-54-121127, JP-A-55-4024, JP-A-55-4025, JP-A-55-29883, JP-A-55-126241, JP-A-55-65955, JP-A-55-65956, JP-A-57-179843, JP-A-54-61125, and West German Patent No. 1045373), polyphenol-based chelating agents, and polyamine-based chelate compounds, with aminopolycarboxylic acid derivatives being particularly preferred.

Preferred examples of the aminopolycarboxylic acid derivative include the compounds shown in the Table attached to "EDTA (-Complexane no Kagaku-) (EDTA—Chemistry of Complexane-)", Nankodo (1977). In these compounds, a 25 part of the carboxyl groups may be substituted by an alkali metal salt, such as sodium or potassium, or by an ammonium salt. More preferred examples of the aminopolycarboxylic acid derivative include iminodiacetic acid, N-methyliminodiacetic acid, N-(2-aminoethyl)iminodiacetic acid, N-(carbamoylmethyl)iminodiacetic acid, nitrilotriacetic acid, ethylenediamine-N,N'-diacetic acid, ethylenediamine-N,N'-di- $\alpha$ -propionic acid, ethylenediamine-N,N'-di- $\beta$ -propionic acid, N,N'-ethylene-bis( $\alpha$ -o-hydroxyphenyl)glycine, N,N'-di(2-hydroxybenzyl)ethylenediamine-N,N'-diacetic acid, ethylenediamine-N,N'-diacetic acid-N,N'-diacetohydroxamic acid, N-hydroxyethyl ethylenediamine-N,N',N'-triacetic acid, ethylenediamine-N,N,N',N'-tetraacetic acid, 1,2-propylenediamine-N,N,N',N'-tetraacetic acid, d,l-2,3-diaminobutane-N,N,N',N'-tetraacetic acid, meso-2,3-diaminobutane-N,N,N',N'-tetraacetic acid, 1-phenylethylenediamine-N,N,N',N'-tetraacetic acid, d,l-1,2-diphenylethylenediamine-N,N,N',N'-tetraacetic acid, 1,4-diaminobutane-N,N,N',N'-tetraacetic acid, trans-cyclobutane-1,2-diamine-N,N,N',N'-tetraacetic acid, trans-cyclopentane-1,2-diamine-N,N,N',N'-tetraacetic acid, cis-cyclohexane-1,2-diamine-N,N,N',N'-tetraacetic acid, cis-cyclohexane-1,3-diamine-N,N,N',N'-tetraacetic acid, cyclohexane-1,4-diamine-N,N,N',N'-tetraacetic acid, o-phenylenediamine-N,N,N',N'-tetraacetic acid, cis-1,4-diaminobutene-N,N,N',N'-tetraacetic acid, trans-1,4-diaminobutene-N,N,N',N'-tetraacetic acid,  $\alpha$ , $\alpha$ '-diamino-o-xylene-N,N,N',N'-tetraacetic acid, 2-hydroxy-1,3-propanediamine-N,N,N',N'-tetraacetic acid, 2,2'-oxy-bis(ethyliminodiacetic acid), 2,2'-ethylenedioxy-bis(ethyliminodiacetic acid), ethylenediamine-N,N'-diacetic acid-N,N'-di- $\alpha$ -propionic acid, ethylenediamine-N,N'-di- $\beta$ -propionic acid, ethylenediamine-N,N,N',N'-tetrapropionic acid, diethylenetriamine-N,N,N',N",N"-pentaacetic acid, triethylenetetramine-N,N,N',N",N"-hexaacetic acid, and 1,2,3-triaminopropane-N,N,N',N",N"-hexaacetic acid. In these compounds, a part of the carboxyl groups may be substituted by an alkali metal salt, such as sodium or potassium, or by an ammonium salt.

The amount of the chelating agent to be added is preferably 0.01 mass % to 0.4 mass %, more preferably 0.02 mass % to 0.3 mass %, and especially preferably 0.03 mass % to 0.15 mass %, based on the total amount of monomers. When the

addition amount of the chelating agent is too small, metal ions entering during the preparation of the latex polymer are not sufficiently trapped, and the stability of the latex against aggregation is lowered, whereby the coating properties become worse. When the amount is too large, the viscosity of the latex increases, whereby the coating properties are lowered.

In the preparation of the latex polymer to be used in the present invention, it is preferable to use a chain transfer agent. As the chain transfer agent, ones described in Polymer Handbook (3rd Edition) (Wiley-Interscience, 1989) are preferable. Sulfur compounds are more preferable because they have high chain-transfer ability and because the amount to be used can be small. Especially, hydrophobic mercaptane-based chain transfer agents, such as tert-dodecylmercaptane and n-dodecylmercaptane, are preferable.

The amount of the chain transfer agent to be added is preferably 0.2 mass % to 2.0 mass %, more preferably 0.3 mass % to 1.8 mass %, and especially preferably 0.4 mass % to 1.6 mass %, based on the total amount of monomers.

Besides the foregoing compounds, in the emulsion polymerization, use can be made of additives, such as electrolytes, stabilizers, thickeners, defoaming agents, antioxidants, vulcanizers, antifreezing agents, gelling agents, and vulcanization accelerators, as described, for example, in "Synthetic Rubber Handbook".

In the present invention, it is preferable to prepare the latex polymer by applying an aqueous type coating solution and then drying it. The "aqueous type" so-called herein means that 60% by mass or more of the solvent (dispersion medium) of the coating solution is water. As a component other than water in the coating solution, a water miscible organic solvent may be used, such as methyl alcohol, ethyl alcohol, isopropyl alcohol, methyl cellosolve, ethyl cellosolve, dimethylformamide, ethyl acetate, diacetone alcohol, furfuryl alcohol, benzyl alcohol, diethylene glycol monoethyl ether, and oxyethyl phenyl ether.

The latex polymer in the image-receiving sheet used in the present invention includes a state of a gel or dried film formed by removing a part of solvents by drying after coating.

<Water-Soluble Polymer>

The receptor layer preferably contains a water-soluble polymer. Herein, "water-soluble polymer" means a polymer which dissolves, in 100 g of water at 20°C., in an amount of preferably 0.05 g or more, more preferably 0.1 g or more, further preferably 0.5 g or more, and particularly preferably 1 g or more. The water-soluble polymer which can be used in the present invention is natural polymers (polysaccharide type, microorganism type, and animal type), semi-synthetic polymers (cellulose-based, starch-based, and alginic acid-based), and synthetic polymer type (vinyl type and others); and synthetic polymers including polyvinyl alcohols, and natural or semi-synthetic polymers using celluloses or the like derived from plant as starting materials, which will be explained later, correspond to the water-soluble polymer usable in the present invention. The latex polymers recited above are not included in the water-soluble polymers which can be used in the present invention.

In the present invention, the water-soluble polymer is also referred to as a binder, for differentiation from the latex polymer described above.

Among the water-soluble polymers which can be used in the present invention, the natural polymers and the semi-synthetic polymers will be explained in detail. Specific examples include the following polymers: plant type polysaccharides, such as gum arabics,  $\kappa$ -carrageenans,  $\iota$ -carrageenans,  $\lambda$ -carrageenans, guar gums (e.g. Supercol, manufactured

by Squalon), locust bean gums, pectins, tragacanths, corn starches (e.g. Purity-21, manufactured by National Starch & Chemical Co.), and phosphorylated starches (e.g. National 78-1898, manufactured by National Starch & Chemical Co.); microbial type polysaccharides, such as xanthan gums (e.g. Keltrol T, manufactured by Kelco), and dextrans (e.g. Nadex 360, manufactured by National Starch & Chemical Co.); animal type natural polymers, such as gelatins (e.g. Crodyne B419, manufactured by Croda), caseins, sodium chondroitin sulfates (e.g. Cromoist CS, manufactured by Croda); cellulose-based polymers, such as ethylcelluloses (e.g. Cellofas WLD, manufactured by I.C.I.), carboxymethylcelluloses (e.g. CMC, manufactured by Daicel), hydroxyethylcelluloses (e.g. HEC, manufactured by Daicel), hydroxypropylcelluloses (e.g. Klucel, manufactured by Aqualon), methylcelluloses (e.g. Viscontran, manufactured by Henkel), nitrocelluloses (e.g. Isopropyl Wet, manufactured by Hercules), and cationated celluloses (e.g. Crodacel QM, manufactured by Croda); starches, such as phosphorylated starches (e.g. National 78-1898, manufactured by National Starch & Chemical Co.); alginic acid-based compounds, such as sodium alginates (e.g. Keltone, manufactured by Kelco), and propylene glycol alginates; and other polymers, such as cationated guar gums (e.g. Hi-care 1000, manufactured by Alcolac), and sodium hyaluronates (e.g. Hyalure, manufactured by Lifecare Biomedical) (all of the names are trade names).

Gelatin is one of preferable embodiments in the present invention. Gelatin having a molecular weight of from 10,000 to 1,000,000 may be used in the present invention. Gelatin that can be used in the present invention may contain an anion, such as  $\text{Cl}^-$  and  $\text{SO}_4^{2-}$ , or a cation, such as  $\text{Fe}^{2+}$ ,  $\text{Ca}^{2+}$ ,  $\text{Mg}^{2+}$ ,  $\text{Sn}^{2+}$ , and  $\text{Zn}^{2+}$ . Gelatin is preferably added as an aqueous solution.

Among the water-soluble polymers which can be used in the present invention, the synthetic polymers will be explained in detail. Examples of the acryl type include sodium polyacrylates, polyacrylic acid copolymers, polyacrylamides, polyacrylamide copolymers, and polydiethylaminoethyl(meth)acrylate quaternary salts or their copolymers. Examples of the vinyl type include polyvinylpyrrolidones, polyvinylpyrrolidone copolymers, and polyvinyl alcohols. Examples of other types include polyethylene glycols, polypropylene glycols, polyisopropylacrylamides, polymethyl vinyl ethers, polyethyleneimines, polystyrenesulfonic acids or their copolymers, naphthalenesulfonic acid condensate salts, polyvinylsulfonic acids or their copolymers, polyacrylic acids or their copolymers, acrylic acid or its copolymers, maleic acid copolymers, maleic acid monoester copolymers, acryloylmethylpropane-sulfonic acid or its copolymers, polydimethylallylammomium chlorides or their copolymers, polyamidines or their copolymers, polyimidazolines, dicyanamide type condensates, epichlorohydrin/dimethylamine condensates, Hoffmann decomposed products of polyacrylamides, and water-soluble polyesters (Plascoat Z-221, Z-446, Z-561, Z-450, Z-565, Z-850, Z-3308, RZ-105, RZ-570, Z-730 and RZ-142 (all of these names are trade names), manufactured by Goo Chemical Co., Ltd.).

In addition, highly-water-absorptive polymers, namely, homopolymers of vinyl monomers having  $-\text{COOM}$  or  $-\text{SO}_3\text{M}$  (M represents a hydrogen atom or an alkali metal atom) or copolymers of these vinyl monomers among them or with other vinyl monomers (for example, sodium methacrylate, ammonium methacrylate, Sumikagel L-5H (trade name) manufactured by Sumitomo Chemical Co., Ltd.) as described in, for example, U.S. Pat. No. 4,960,681 and JP-A-62-245260, may also be used.

Among the water-soluble synthetic polymers that can be used in the present invention, polyvinyl alcohols are preferable.

The polyvinyl alcohols are explained in detail below.

Examples of completely saponified polyvinyl alcohol include PVA-105 [polyvinyl alcohol (PVA) content: 94.0 mass % or more; degree of saponification:  $98.5\pm0.5$  mol %; content of sodium acetate: 1.5 mass % or less; volatile constituent: 5.0 mass % or less; viscosity (4 mass %; 20° C.):  $5.6\pm0.4$  CPS]; PVA-110 [PVA content: 94.0 mass %; degree of saponification:  $98.5\pm0.5$  mol %; content of sodium acetate: 1.5 mass %; volatile constituent: 5.0 mass %; viscosity (4 mass %; 20° C.):  $11.0\pm0.8$  CPS]; PVA-117 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.):  $28.0\pm3.0$  CPS]; PVA-117H [PVA content: 93.5 mass %; degree of saponification:  $99.6\pm0.3$  mol %; content of sodium acetate: 1.85 mass %; volatile constituent: 5.0 mass %; viscosity (4 mass %; 20° C.):  $29.0\pm3.0$  CPS]; PVA-120 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.):  $39.5\pm4.5$  CPS]; PVA-124 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.):  $60.0\pm6.0$  CPS]; PVA-124H [PVA content: 93.5 mass %; degree of saponification:  $99.6\pm0.3$  mol %; content of sodium acetate: 1.85 mass %; volatile constituent: 5.0 mass %; viscosity (4 mass %; 20° C.):  $61.0\pm6.0$  CPS]; PVA-CS [PVA content: 94.0 mass %; degree of saponification:  $97.5\pm0.5$  mol %; content of sodium acetate: 1.0 mass %; volatile constituent: 5.0 mass %; viscosity (4 mass %; 20° C.):  $27.5\pm3.0$  CPS]; PVA-CST [PVA content: 94.0 mass %; degree of saponification:  $96.0\pm0.5$  mol %; content of sodium acetate: 1.0 mass %; volatile constituent: 5.0 mass %; viscosity (4 mass %; 20° C.):  $27.0\pm3.0$  CPS]; and PVA-HC [PVA content: 90.0 mass %; degree of saponification: 99.85 mol % or more; content of sodium acetate: 2.5 mass %; volatile constituent: 8.5 mass %; viscosity (4 mass %; 20° C.):  $25.0\pm3.5$  CPS] (all trade names, manufactured by Kuraray Co., Ltd.), and the like.

Examples of partially saponified polyvinyl alcohol include PVA-203 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $3.4\pm0.2$  CPS]; PVA-204 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $3.9\pm0.3$  CPS]; PVA-205 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $5.0\pm0.4$  CPS]; PVA-210 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $9.0\pm1.0$  CPS]; PVA-217 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $22.5\pm2.0$  CPS]; PVA-220 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $30.0\pm3.0$  CPS]; PVA-224 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $44.0\pm4.0$  CPS]; PVA-228 [PVA content: 94.0 mass %; degree of saponification:  $88.0\pm1.5$  mol %; content of sodium acetate:

1.0 mass %; volatile constituent: 5.0 mass %; viscosity (4 mass %; 20° C.):  $65.0\pm5.0$  CPS]; PVA-235 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $95.0\pm15.0$  CPS]; PVA-217EE [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $23.0\pm3.0$  CPS]; PVA-217E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $23.0\pm3.0$  CPS]; PVA-220E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $31.0\pm4.0$  CPS]; PVA-224E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $45.0\pm5.0$  CPS]; PVA-403 [PVA content: 94.0 mass %; degree of saponification:  $80.0\pm1.5$  mol %; content of sodium acetate: 1.0 mass %; volatile constituent: 5.0 mass %; viscosity (4 mass %; 20° C.):  $3.1\pm0.3$  CPS]; PVA-405 [PVA content: 94.0 mass %; degree of saponification:  $81.5\pm1.5$  mol %; content of sodium acetate: 1.0 mass %; volatile constituent: 5.0 mass %; viscosity (4 mass %; 20° C.):  $4.8\pm0.4$  CPS]; PVA-420 [PVA content: 94.0 mass %; degree of saponification:  $79.5\pm1.5$  mol %; content of sodium acetate: 1.0 mass %; volatile constituent: 5.0 mass %]; PVA-613 [PVA content: 94.0 mass %; degree of saponification:  $93.5\pm1.0$  mol %; content of sodium acetate: 1.0 mass %; volatile constituent: 5.0 mass %; viscosity (4 mass %; 20° C.):  $16.5\pm2.0$  CPS]; L-8 [PVA content: 96.0 mass %; degree of saponification:  $71.0\pm1.5$  mol %; content of sodium acetate: 1.0 mass % (ash); volatile constituent: 3.0 mass %; viscosity (4 mass %; 20° C.):  $5.4\pm0.4$  CPS] (all trade names, manufactured by Kuraray Co., Ltd.), and the like.

The above values measured were determined according to JIS K-6726-1977.

With respect to modified polyvinyl alcohols, those described by Koichi Nagano, et al., "Poval", issued by Kobunshi Kankokai, Inc. can be used. The modified-polyvinyl alcohols include polyvinyl alcohols modified by cations, anions, —SH compounds, alkylthio compounds, or silanols.

Examples of such modified polyvinyl alcohols (modified PVA) include C polymers, such as C-118, C-318, C-318-2A, and C-506 (all being trade names of Kuraray Co., Ltd.); HL polymers, such as HL-12E and HL-1203 (all being trade names of Kuraray Co., Ltd.); HM polymers, such as HM-03 and HM-N-03 (all being trade names of Kuraray Co., Ltd.); K polymers, such as KL-118, KL-318, KL-506, KM-118T, and KM-618 (all being trade names of Kuraray Co., Ltd.); M polymers, such as M-115 (a trade name of Kuraray co., Ltd.); MP polymers, such as MP-102, MP-202, and MP-203 (all being trade names of Kuraray Co., Ltd.); MPK polymers, such as MPK-1, MPK-2, MPK-3, MPK-4, MPK-5, and MPK-6 (all being trade names of Kuraray Co., Ltd.); R polymers, such as R-1130, R-2105, and R-2130 (all being trade names of Kuraray Co., Ltd.); and V polymers, such as V-2250 (a trade name of Kuraray Co., Ltd.).

The viscosity of polyvinyl alcohol can be adjusted or stabilized by adding a trace amount of a solvent or an inorganic salt to an aqueous solution of polyvinyl alcohol, and use may be made of a compound, as described in the aforementioned reference "Poval", Koichi Nagano et al., published by Kobunshi Kankokai, pp. 144-154. For example, a coated-surface quality can be improved by an addition of boric acid, and the

addition of boric acid is preferable. The amount of boric acid to be added is preferably 0.01 to 40 mass % with respect to polyvinyl alcohol.

Preferred binders are transparent or semitransparent, and generally colorless. Examples thereof include natural resins, polymers and copolymers; synthetic resins, polymers, and copolymers; and other media that form films: for example, rubbers, polyvinyl alcohols, hydroxyethyl celluloses, cellulose acetates, cellulose acetate butylates, polyvinylpyrrolidones, starches, polyacrylic acids, polymethyl methacrylates, polyvinyl chlorides, polymethacrylic acids, styrene/maleic acid anhydride copolymers, styrene/acrylonitrile copolymers, styrene/butadiene copolymers, polyvinylacetals (e.g., polyvinylformals and polyvinylbutyral), polyesters, polyurethanes, phenoxy resins, polyvinylidene chlorides, polyepoxides, polycarbonates, polyvinyl acetates, polyolefins, cellulose esters, and polyamides. These media are water-soluble.

In the present invention, preferred water-soluble polymers are polyvinyl alcohols and gelatin, with gelatin being most preferred.

The amount of the water-soluble polymer to be added to the receptor layer is preferably from 1 to 25% by mass, more preferably from 1 to 10% by mass, based on the entire mass of the receptor layer.

<Hardener>

As a crosslinking agent (compound capable of crosslinking, for example, a water-soluble polymer), a hardener (hardening agent) may be added in a coating layer(s) (e.g., the receptor layer, the heat insulation layer, the undercoat layer) of the image-receiving sheet of the present invention.

The receptor layer preferably contains a crosslinking agent.

A part or all of the above-mentioned water-soluble polymer contained in the receptor layer has been preferably crosslinked with the crosslinking agent.

Preferred examples of the hardener that can be used in the present invention include H-1, 4, 6, 8, and 14 in JP-A-1-214845 in page 17; compounds (H-1 to H-54) represented by one of the formulae (VII) to (XII) in U.S. Pat. No. 4,618,573, columns 13 to 23; compounds (H-1 to H-76) represented by the formula (6) in JP-A-2-214852, page 8, the lower right (particularly, H-14); and compounds described in claim 1 in U.S. Pat. No. 3,325,287. Examples of the hardening agent include hardening agents described, for example, in U.S. Pat. No. 4,678,739, column 41, U.S. Pat. No. 4,791,042, JP-A-59-116655, JP-A-62-245261, JP-A-61-18942, and JP-A-4-

218044. More specifically, an aldehyde-series hardening agent (formaldehyde, etc.), an aziridine-series hardening agent, an epoxy-series hardening agent, a vinyl sulfone-series hardening agent (N,N'-ethylene-bis(vinylsulfonylacetamido) ethane, etc.), an N-methylol-series hardening agent (dimethylol urea, etc.), boric acid, metaboric acid, or a polymer hardening agent (compounds described, for example, in JP-A-62-234157), can be mentioned.

Preferred examples of the hardener include a vinylsulfone-series hardener and chlorotriazines.

More preferable hardeners in the present invention are compounds represented by the following formula (B) or (C).



In formulae (B) and (C), X represents a halogen atom, L represents an organic linking group having n-valency. When the compound represented by formula (B) or (C) is a low-molecular compound, n denotes an integer of from 1 to 4.

When the compound represented by formula (B) or (C) is a high-molecular (polymer) compound, L represents an organic linking group containing a polymer chain, and n denotes an integer within the range of from 10 to 1,000.

In the formulae (B) and (C), X is preferably a chlorine atom or a bromine atom, and further preferably a bromine atom. n is an integer of from 1 to 4, preferably an integer of from 2 to 4, more preferably 2 or 3, and most preferably 2.

L represents an organic group having n-valency, and preferably an aliphatic hydrocarbon group, an aromatic hydrocarbon group, or a heterocyclic group, in which these groups may be further linked through an ether bond, ester bond, amide bond, sulfonamide bond, urea bond, urethane bond, or the like. Also, each of these groups may have a substituent. Examples of the substituent include a halogen atom, an alkyl group, an aryl group, a heterocyclic group, a hydroxyl group, an alkoxy group, an aryloxy group, an alkylthio group, an arylthio group, an acyloxy group, an alkoxy carbonyl group, a carbamoyloxy group, an acyl group, an acyloxy group, an acylamino group, a sulfonamido group, a carbamoyl group, a sulfamoyl group, a sulfonyl group, a phosphoryl group, a carboxyl group, and a sulfo group. Among these groups, a halogen atom, an alkyl group, a hydroxy group, an alkoxy group, an aryloxy group, and an acyloxy group are preferable.

Specific examples of the vinylsulfone-series hardener include the following compounds (VS-1) to (VS-27), but not limited to those in the present invention.



-continued  
(VS-11)

These hardeners may be obtained with reference to the method described in, for example, U.S. Pat. No. 4,173,481.

Furthermore, as the chlorotriazine-series hardener, a 1,3,5-triazine compound in which at least one of the 2-position, 4-position and 6-position of the triazine ring in the compound is substituted with a chlorine atom, is preferable. A 1,3,5-triazine compound in which two or three of the 2-position, 4-position and 6-position of the triazine ring each are substituted with a chlorine atom, is more preferable. Alternatively, use may be made of a 1,3,5-triazine compound in which at least one of the 2-position, 4-position and 6-position of the triazine ring is substituted with a chlorine atom, and the remainder position(s) is/are substituted with a group(s) or atom(s) other than a chlorine atom. Examples of the group or atom other than chlorine atom include a hydrogen atom, a bromine atom, a fluorine atom, an iodine atom, an alkyl group, an alkenyl group, an alkynyl group, a cycloalkyl

group, a cycloalkenyl group, an aryl group, a heterocyclic group, a hydroxy group, a nitro group, a cyano group, an amino group, a hydroxylamino group, an alkylamino group, an arylamino group, a heterocyclic amino group, an acylamino group, a sulfonamido group, a carbamoyl group, a sulfamoyl group, a sulfo group, a carboxyl group, an alkoxy group, an alkenoxy group, an aryloxy group, a heterocyclic oxy group, an acyl group, an acyloxy group, an alkyl- or aryl-sulfonyl group, an alkyl- or aryl-sulfinyl group, an alkyl- or aryl-sulfonyloxy group, a mercapto group, an alkylthio group, an alkenylthio group, an arylthio group, a heterocyclic thio group, and an alkyloxy- or aryloxy-carbonyl group.

Specific examples of the chlorotriazine-series hardener include 4,6-dichloro-2-hydroxy-1,3,5-triazine or its Na salt, 2-chloro-4,6-diphenoxypyrimidine, 2-chloro-4,6-bis[2,4,6-trimethylphenoxy]triazine, 2-chloro-4,6-diglycidoxo-1,3,5-triazine, 2-chloro-4-(n-butoxy)-6-glycidoxo-1,3,5-triazine,



21

2-chloro-4-(2,4,6-trimethylphenoxy)-6-glycidoxy-1,3,5-triazine, 2-chloro-4-(2-chloroethoxy)-6-(2,4,6-trimethylphenoxy)-1,3,5-triazine, 2-chloro-4-(2-bromoethoxy)-6-(2,4,6-trimethylphenoxy)-1,3,5-triazine, 2-chloro-4-(2-di-n-butylphosphatoethoxy)-6-(2,4,6-trimethylphenoxy)-1,3,5-triazine, and 2-chloro-4-(2-di-n-butylphosphatoethoxy)-6-(2,6-xylenoxy)-1,3,5-triazine, but the present invention is not limited to those.

Such a compound can be easily produced by reacting cyanur chloride (namely, 2,4,6-trichlorotriazine) with, for example, a hydroxy compound, thio compound or amino compound corresponding to the substituent to be introduced on the heterocycle.

These hardeners are used in an amount of generally 0.001 to 1 g, preferably 0.005 to 0.5 g, per g of the water-soluble polymer.

## &lt;Emulsion&gt;

An emulsion is preferably incorporated in the receptor layer of the heat-sensitive transfer image-receiving sheet of the present invention. The following is a detailed explanation of the emulsion that can be preferably used in the present invention.

A hydrophobic additive(s), such as a lubricant, an antioxidant, and the like, can be introduced into a layer of the image-receiving sheet (e.g. the receptor layer, the heat insulation layer, the undercoat layer), by using a known method described in U.S. Pat. No. 2,322,027, or the like. In this case, a high-boiling organic solvent, as described in U.S. Pat. Nos. 4,555,470, 4,536,466, 4,536,467, 4,587,206, 4,555,476 and 4,599,296, JP-B-3-62256, and the like, may be used singly or in combination with a low-boiling organic solvent having a boiling point of 50 to 160° C., according to the need. Also, these lubricants, antioxidants, and high-boiling organic solvents may be respectively used singly or in combination of two or more thereof.

As the antioxidant (hereinafter, also referred to as a radical trapper in this specification), a compound represented by any one of the following formulae (E-1) to (E-3) can be preferably used.

Formula (E-1)



Formula (E-2)



22

-continued

Formula (E-3)



R<sub>41</sub> represents an aliphatic group, an aryl group, a heterocyclic group, an acyl group, an aliphatic oxycarbonyl group, an aryloxycarbonyl group, an aliphatic sulfonyl group, an arylsulfonyl group, a phosphoryl group, or a group —Si(R<sub>47</sub>)(R<sub>48</sub>)(R<sub>49</sub>), in which R<sub>47</sub>, R<sub>48</sub> and R<sub>49</sub> each independently represent an aliphatic group, an aryl group, an aliphatic oxy group, or an aryloxy group. R<sub>42</sub>, R<sub>43</sub>, R<sub>45</sub>, and R<sub>46</sub> each independently represent a hydrogen atom or a substituent. Examples of the substituent include a halogen atom, an aliphatic group (include an alkyl group, an alkenyl group, an alkynyl group, a cycloalkyl group, a cycloalkenyl group), an aryl group, a heterocyclic group, a hydroxy group, a mercapto group, an aliphatic oxy group, an aryloxy group, a heterocyclic oxy group, an aliphatic thio group, an arylthio group, a heterocyclic thio group, an amino group, an aliphatic amino group, an arylamino group, a heterocyclic amino group, an acylamino group, a sulfonamido group, a cyano group, a nitro group, a carbamoyl group, a sulfamoyl group, an acyl group, an aliphatic oxy carbonyl group, or an aryloxy carbonyl group. R<sub>a1</sub>, R<sub>a2</sub>, R<sub>a3</sub>, and R<sub>a4</sub> each independently represent a hydrogen atom or an aliphatic group (for example, methyl, ethyl).

With respect to the compounds represented by any one of the formulae (E-1) to (E-3), the groups that are preferred from the viewpoint of the effect to be obtained by the present invention, are explained below.

In the formulae (E-1) to (E-3), it is preferred that R<sub>41</sub> represents an aliphatic group, an acyl group, an aliphatic oxycarbonyl group, an aryloxycarbonyl group, or a phosphoryl group, and R<sub>42</sub>, R<sub>43</sub>, R<sub>45</sub>, and R<sub>46</sub> each independently represent a hydrogen atom, an aliphatic group, an aliphatic oxy group, or an acylamino group. It is more preferred that R<sub>41</sub> represents an aliphatic group, and R<sub>42</sub>, R<sub>43</sub>, R<sub>45</sub> and R<sub>46</sub> each independently represent a hydrogen atom or an aliphatic group.

Preferred specific examples of the compounds represented by any one of the formulae (E-1) to (E-3) are shown below, but the present invention is not limited to these compounds.

EB-1



**23**

-continued

**24**

-continued

EB-2



EB-3



EB-4



EB-5



EB-6

As the lubricant, solid waxes, such as polyethylene wax, amide wax, and Teflon (registered trademark) powder; silicone oil, phosphate-series compounds, fluorine-based surfactants, silicone-based surfactants, and others including releasing agents known in the technical fields of the art concerned may be used. Fluorine-series compounds typified by fluorine-based surfactants, and silicone-series compounds, such as silicone-based surfactants and silicone oil and/or its hardened products, are preferably used. A content of the lubricant is preferably from 1.0 to 10.0 mass %, more preferably from 1.5 to 2.5 mass %, based on a solid content in the latex polymer.

As the silicone oil as the lubricant, straight silicone oil and modified silicone oil or their hardened products may be used.

Examples of the straight silicone oil include dimethylsilicone oil, methylphenylsilicone oil, and methyl hydrogen silicone oil. Examples of the dimethylsilicone oil include KF96-10, KF96-100, KF96-1000, KF96H-10000, KF96H-12500, and KF96H-100000 (all of these names are trade names, manufactured by Shin-Etsu Chemical Co., Ltd.). Examples of the methylphenylsilicone oil include KF50-100, KF54, and KF56 (all of these names are trade names, manufactured by Shin-Etsu Chemical Co., Ltd.).

The modified silicone oil may be classified into reactive silicone oils and non-reactive silicone oils. Examples of the reactive silicone oils include amino-modified, epoxy-modified, carboxyl-modified, hydroxy-modified, methacryl-

EB-8

EB-9

EB-10

EB-11

25

modified, mercapto-modified, phenol-modified, or one-terminal reactive/hetero-functional group-modified silicone oils. Examples of the amino-modified silicone oil include KF-393, KF-857, KF-858, X-22-3680, X-22-3801C, KF-8010, X-22-161A, and KF-8012 (all of these names are trade names, manufactured by Shin-Etsu Chemical Co., Ltd.). Examples of the epoxy-modified silicone oil include KF-100T, KF-101, KF-60-164, KF-103, X-22-343, and X-22-3000T (all of these names are trade names, manufactured by Shin-Etsu Chemical Co., Ltd.). Examples of the carboxyl-modified silicone oil include X-22-162C (trade name, manufactured by Shin-Etsu Chemical Co., Ltd.). Examples of the hydroxy-modified silicone oil include X-22-160AS, KF-6001, KF-6002, KF-6003, X-22-170DX, X-22-176DX, X-22-176D, and X-22-176DF (all of these names are trade names, manufactured by Shin-Etsu Chemical Co., Ltd.). Examples of the methacryl-modified silicone oil include X-22-164A, X-22-164C, X-24-8201, X-22-174D, and X-22-2426 (all of these names are trade names, manufactured by Shin-Etsu Chemical Co., Ltd.).

Reactive silicone oils may be hardened upon use, and may be classified into a reaction-curable type, photocurable type, catalyst-curable type, and the like. Among these types, silicone oil that is the reaction-curable type is particularly preferable. As the reaction-curable type silicone oil, products obtained by allowing an amino-modified silicone oil to react with an epoxy-modified silicone oil, followed by curing the resultant reaction product, are preferable. Also, examples of the catalyst-curable type or photocurable type silicone oil include KS-705F-PS, KS-705F-PS-1, and KS-770-PL-3 (all of these names are trade names, catalyst-curable silicone oils, manufactured by Shin-Etsu Chemical Co., Ltd.), and KS-720 and KS-774-PL-3 (all of these names are trade names, photocurable-type silicone oils, manufactured by Shin-Etsu Chemical Co., Ltd.). The addition amount of the curable type silicone oil is preferably 0.5 to 30% by mass based on the resin constituting the receptor layer. The releasing agent is used in an amount of generally about 2 to 4 parts by mass, preferably about 2 to 3 parts by mass, based on 100 parts by mass of the polyester resin. If the amount is too small, the releasing property cannot be secured without fail, whereas if the amount is too large, a protective layer is not transferred to the image-receiving sheet resultantly.

Examples of the non-reactive silicone oil include polyether-modified, methylstyryl-modified, alkyl-modified, higher fatty acid ester-modified, hydrophilic special-modified, higher alkoxy-modified, or fluorine-modified silicone oils. Examples of the polyether-modified silicone oil include KF-6012 (trade name, manufactured by Shin-Etsu Chemical Co., Ltd.), and examples of the methylstyryl-modified silicone oil include 24-510, and KF41-410 (all of these names are trade names, manufactured by Shin-Etsu Chemical Co., Ltd.). Modified silicones represented by any one of the following formulae 1 to 3 may also be used.

Formula 1



26

In formula 1, R represents a hydrogen atom, or a straight-chain or branched alkyl group which may be substituted with an aryl or cycloalkyl group. m and n each denote an integer of 2,000 or less, and a and b each denote an integer of 30 or less.

Formula 2



Formula 3



In formula 3, R represents a hydrogen atom, or a straight-chain or branched alkyl group which may be substituted with an aryl or cycloalkyl group. m and n each denote an integer of 2,000 or less, and a and b each denote an integer of 30 or less.

$\text{R}^1$  represents a single bond or a divalent linking group, E represents an ethylene group which may be further substituted, and P represents a propylene group which may be further substituted.

Silicone oils such as those mentioned above are described in "SILICONE HANDBOOK" (The Nikkan Kogyo Shim bun, Ltd.), and the techniques described in each publication of JP-A-8-108636 and JP-A-2002-264543 may be preferably used as the techniques to cure the curable type silicone oils.

Examples of the high-boiling organic solvent include phthalates (e.g., dibutyl phthalate, dioctyl phthalate, di-2-ethylhexyl phthalate), phosphates or phosphonates (e.g., triphenyl phosphate, tricresyl phosphate, tri-2-ethylhexyl phosphate), fatty acid esters (e.g., di-2-ethylhexyl succinate, tributyl citrate), benzoates (e.g., 2-ethylhexyl benzoate, dodecyl benzoate), amides (e.g., N,N-diethyldodecaneamide, N,N-dimethyloleinamide), alcohols or phenols (e.g., isostearyl alcohol, 2,4-di-tert-amyl phenol), anilines (e.g., N,N-dibutyl-2-butoxy-5-tert-octylaniline), chlorinated paraffins, hydrocarbons (e.g., dodecylbenzene, diisopropylnaphthalene), and carboxylic acids (e.g., 2-(2,4-di-tert-amylphenoxy)butyrate).

Preferably, any of the compounds shown below is used.

(Solv-1)



-continued



Further, the high-boiling organic solvent may be used in combination with, as an auxiliary solvent, an organic solvent having a boiling point of 30° C. or more and 160° C. or less, such as ethyl acetate, butyl acetate, methyl ethyl ketone, cyclohexanone, methylcellosolve acetate, or the like. The high-boiling organic solvent is used in an amount of generally 10 g or less, preferably 5 g or less, and more preferably 1 to 0.1 g, per g of the hydrophobic additive(s) to be used. The amount is also preferably 1 ml or less, more preferably 0.5 ml or less, and particularly preferably 0.3 ml or less, per g of the binder.

A dispersion method that uses a polymer, as described in JP-B-51-39853 and JP-A-51-59943, and a method in which the addition is made with those substances in the form of a dispersion of fine particles thereof, as described in, for example, JP-A-62-30242, can also be used. In the case of a compound that is substantially insoluble in water, other than the above methods, a method can be used in which the compound is dispersed and contained in the form of fine particles thereof in a binder.

When the hydrophobic compound is dispersed in a hydrophilic colloid, various surfactants may be used. For example, those listed as examples of the surfactant in JP-A-59-157636, page (37) to page (38) may be used. It is also possible to use phosphates-based surfactants described in JP-A-7-56267, JP-A-7-228589, and West German Patent Application Laid-Open (OLS) No. 1,932,299A.

<Ultraviolet Absorber>

Further, in the present invention, in order to improve light resistance, an ultraviolet absorber may be added to the recep-

tor layer. In this case, when this ultraviolet absorber is made to have a higher molecular weight, the resultant UV absorber can be secured (immobilized) to the receptor layer so that the UV absorber can be prevented, for instance, from being diffused into the ink sheet or from being sublimated/vaporized by heating.

As the ultraviolet absorber, compounds having various ultraviolet absorber skeletons, which are widely known in the field of information recording, may be used. Specific examples of the ultraviolet absorber include compounds having a 2-hydroxybenzotriazole type ultraviolet absorber skeleton, 2-hydroxybenzotriazine type ultraviolet absorber skeleton, or 2-hydroxybenzophenone type ultraviolet absorber skeleton. Compounds having a benzotriazole-type or triazine-type skeleton are preferable, from the viewpoint of ultraviolet absorbing ability (absorption coefficient) and stability; and compounds having a benzotriazole-type or benzophenone-type skeleton are preferable, from the viewpoint of obtaining a higher-molecular weight and using in a form of a latex. Specifically, ultraviolet absorbers described in, for example, JP-A-2004-361936 may be used.

The ultraviolet absorber preferably absorbs light at wavelengths in the ultraviolet region, and the absorption edge of the absorption of the ultraviolet absorber is preferably out of the visible region. Specifically, when the UV absorber is added to the receptor layer to form a heat-sensitive transfer image-receiving sheet, the resultant heat-sensitive transfer image-receiving sheet has a reflection density of, preferably, Abs 0.5 or more at 370 nm, and more preferably Abs 0.5 or more at 380 nm. Also, the heat-sensitive transfer image-receiving sheet has a reflection density of, preferably, Abs 0.1 or less at 400 nm. If the reflection density at a wavelength range exceeding 400 nm is too high, it is not preferable because an image is made yellowish.

In the present invention, the ultraviolet absorber is preferably made to have a higher molecular weight. The ultraviolet absorber has a mass average molecular weight of preferably 10,000 or more, and more preferably 100,000 or more. As a means of obtaining a higher-molecular weight ultraviolet absorber, it is preferable to graft an ultraviolet absorber on a polymer. The polymer as the principal chain preferably has a polymer skeleton less capable of being dyed than the receptor polymer to be used together. Also, when the polymer is made into a form of a film, the film preferably has sufficient film strength. The graft ratio of the ultraviolet absorber to the polymer principal chain is preferably 5 to 20% by mass, and more preferably 8 to 15% by mass.

Also, it is more preferable that the ultraviolet-absorber-grafted polymer is made into a form of a latex upon using. When the polymer is made into a form of a latex, an aqueous dispersion-system coating solution may be used in application and coating to form the receptor layer, and this enables reduction of the production costs. As a method of making the latex polymer (or making the polymer latex-wise), a method described in, for example, Japanese Patent No. 3450339 may be used. As the ultraviolet absorber to be used in a form of a latex, the following commercially available ultraviolet absorbers may be used, examples of which include ULS-700, ULS-1700, ULS-1383MA, ULS-1635 MH, XL-7016, ULS-933LP, and ULS-935LH, manufactured by Ipposha Oil Industries Co., Ltd.; and New Coat UVA-1025W, New Coat UVA-204W, and New Coat UVA-4512M, manufactured by Shin-Nakamura Chemical Co., Ltd. (all of these names are trade names).

In the case of using an ultraviolet-absorber-grafted polymer in a form of a latex, it may be mixed with a latex of the receptor polymer capable of being dyed, and the resulting mixture is coated. By doing so, a receptor layer, in which the ultraviolet absorber is homogeneously dispersed, can be formed.

The addition amount of the ultraviolet-absorber-grafted polymer or its latex is preferably 5 to 50 parts by mass, and more preferably 10 to 30 parts by mass, to 100 parts by mass of the receptor polymer in a form of latex, which is capable of being dyed to be used to form the receptor layer.

<Releasing Agent>

Further, a releasing agent may be incorporated in the receptor layer, in order to prevent thermal fusion with the heat-sensitive transfer sheet upon image formation. As the releasing agent, a silicone oil, a phosphate-based plasticizer, a fluorine-series compound, or various wax dispersions may be used, and the silicone oil and the wax dispersions are particularly preferably used.

As the silicone oil, modified silicone oil, such as epoxy-modified, alkyl-modified, amino-modified, carboxyl-modified, alcohol-modified, fluorine-modified, alkyl aralkyl polyether-modified, epoxy/polyether-modified, or polyether-modified silicone oil, is preferably used. Among these, a reaction product between vinyl-modified silicone oil and hydrogen-modified silicone oil is preferable. The amount of the releasing agent to be added is preferably 0.2 to 30 parts by mass, per 100 parts by mass of the receptor polymer.

As the wax dispersions, known dispersions may be used. In the present invention, "wax" means an organic substance having an alkyl chain that is in a solid or semisolid state at room temperature (according to the definition given in "Kaitai Wax no Seishitsu to Oyo (Revised edition, Properties and Applications of Wax)", Saiwai Shobo (1989)). Preferable examples of the organic compound include candelilla wax, carnauba wax, rice wax, haze wax, montan wax, ozokerite, paraffin wax, microcrystalline wax, petrodatum, Fischer-Tropsch wax, polyethylene wax, montan wax derivatives, paraffin wax derivatives, microcrystalline wax derivatives, hydrogenated ricinus, hydrogenated ricinus derivatives, 12-hydroxystearic acid, stearic acid amide, phthalic anhydride imide, chlorinated hydrocarbons, and other mixed waxes. Of these waxes, carnauba wax, montan wax and derivatives thereof, paraffin wax and derivatives thereof, microcrystalline wax and derivatives thereof, polyethylene wax, and stearic acid amide are preferred; carnauba wax, montan wax and derivatives thereof, microcrystalline wax, and stearic acid amide are more preferred; and montan wax and derivatives thereof, and microcrystalline wax are further preferred.

These waxes are selected from waxes having melting points of generally 25° C. to 120° C., preferably 40° C. to 100° C., more preferably 60° C. to 90° C.

The wax is preferably in a state of being dispersed in water, more preferably in the form of fine particles. Dispersing waxes in water and forming waxes into fine particles can be performed using the methods as described in the above "Revised version, Properties and Applications of Wax", Saiwai Shobo (1989).

The addition amount of wax is preferably from 0.5 to 30% by mass, more preferably from 1 to 20% by mass, and further preferably from 1.5 to 15% by mass, of the amount of total solid content in the receptor layer.

The amount of the receptor layer to be applied is preferably 0.5 to 10 g/m<sup>2</sup> (solid basis, hereinafter, the amount to be applied in the present specification means a value on solid basis, unless otherwise specified), more preferably 1 to 8

g/m<sup>2</sup>, and further preferably 2 to 7 g/m<sup>2</sup>. The film thickness of the receptor layer is preferably 1 to 20 µm. (Heat Insulation Layer)

A heat insulation layer serves to protect the support from heat when a thermal head or the like is utilized to carry out a transfer operation under heating. Also, because the heat insulation layer has high cushion properties, a heat-sensitive transfer image-receiving sheet having high printing sensitivity can be obtained even in the case of using paper as a substrate (support). The heat insulation layer may be a single layer, or multi-layers. The heat insulation layer is generally provided at a position nearer to the support than the receptor layer.

In the image-receiving sheet of the present invention, the heat insulation layer contains hollow polymer particles.

The hollow polymer particles in the present invention are polymer particles having independent pores inside of the particles. Examples of the hollow polymer particles include (1) non-foaming type hollow particles obtained in the following manner: a dispersion medium, such as water, is contained inside of a capsule wall formed of a polystyrene, acryl resin, or styrene/acryl resin, and, after the resultant coating solution is applied and dried, the dispersion medium in the particles is vaporized out of the particles, with the result that the inside of each particle is made to be hollow; (2) foaming type microballoons obtained in the following manner: a low-boiling point liquid, such as butane and pentane, is encapsulated in a resin composed of any one of polyvinylidene chloride, polyacrylonitrile, polyacrylic acid, polyacrylate, and the mixture or polymer thereof, and after the resultant resin coating material is applied, it is heated to make the low-boiling point liquid expand inside of the particles, whereby the inside of each particle is made to be hollow; and (3) microballoons obtained by foaming the above (2) under heating in advance to foam, thereby to make hollow polymer particles.

The particle size of the hollow polymer particles is preferably 0.1 to 20 µm, more preferably 0.1 to 2 µm, further preferably 0.1 to 1 µm, particularly preferably 0.2 to 0.8 µm. If the particle size is too small, the resultant particles tend to have a smaller hollow ratio, which may cause it impossible to obtain a desired heat-insulation property; whereas, if the particle size is too large, such hollow polymer particles having the particle size too large in relation to the film thickness of the heat insulation layer, may cause it difficult to provide a smooth surface and may tend to cause coating troubles due to the coarse particles.

These hollow polymer particles preferably have a hollow ratio of about 20 to 70%, more preferably 20 to 50%. With a too small hollow ratio, it cannot give a sufficient heat-insulating efficiency; while with an excessively large hollow ratio for the hollow particles that have the above-described preferable particle diameter, imperfect hollow particles increase, with prohibiting sufficient film strength.

The "hollow ratio" of the hollow polymer particles as referred to here is a value P calculated according to formula (a), based on the transmission image photographed by a transmission micrograph of hollow particles.

$$P = \left\{ 1/n \times \sum_{i=1}^n (Rai / Rbi)^3 \right\} \times 100(%) \quad \text{Formula (a)}$$

In formula (a), Rai represents the circle-equivalent diameter of the inner periphery (which shows the periphery of a hollow portion), among two peripheries constituting an image of a specific particle i; Rbi represents the circle-equiva-

lent diameter of the outer periphery (which shows the outer shape of a particle in interest), among the two peripheries constituting the image of the specific particle i; and n is the number of measured particles, and n is generally 300 or more. Herein, the term "circle-equivalent diameter" means the diameter of a circle having an area equivalent to the (projected) area that the hollow portion's periphery or the particle's outer shape has.

The glass transition temperature ( $T_g$ ) of the hollow polymer particles is preferably 70° C. or more, and more preferably 100° C. or more. These hollow polymer particles may be used in combinations of two or more kinds thereof, if necessary.

Such hollow polymer particles are commercially available. Specific examples of the above (1) include Rohpake 1055, manufactured by Rohm and Haas Co.; Boncoat PP-1000, manufactured by Dainippon Ink and Chemicals, Incorporated; SX866(B), manufactured by JSR Corporation; and Nippol MH5055, manufactured by Nippon Zeon (all of these product names are trade names). Specific examples of the above (2) include F-30 and F-50, manufactured by Matsuno Yushi-Seiyaku Co., Ltd. (all of these product names are trade names). Specific examples of the above (3) include F-30E, manufactured by Matsumoto Yushi-Seiyaku Co., Ltd; and Expance 461DE, 551DE, and 551DE20, manufactured by Nippon Ferrite (all of these product names are trade names). Among these, the hollow polymer particles of the series of the aforementioned (1) can be more preferably used. It is particularly preferable that the hollow polymer particles for use in the heat insulation layer may be used in a form of a latex.

A water-dispersible type resin or water-soluble type resin is preferably contained, as a binder, in the heat insulation layer containing the hollow polymer particles. As the binder resin that can be used in the present invention, known resins may be used, for example, acryl resin, styrene/acryl copolymer, polystyrene resin, polyvinyl alcohol resin, vinyl acetate resin, ethylene/vinyl acetate copolymer, vinyl chloride/vinyl acetate copolymer, styrene/butadiene copolymer, polyvinylidene chloride resin, cellulose derivative, casein, starch, and gelatin. Also, these resins may be used either singly or as mixtures of two or more thereof.

The solid content of the hollow polymer particles in the heat insulation layer preferably falls in a range from 5 to 2,000 parts by mass, more preferably 5 to 1,000 parts by mass, and further preferably 5 to 400 parts by mass, assuming that the solid content of the binder resin be 100 parts by mass. The solid content of the hollow polymer particles is preferably 50% by mass or more, more preferably 60% by mass or more, and further preferably 65% by mass or more, based on the total solid content of the hollow polymer particles and the binder resin. Also, the ratio by mass of the solid content of the hollow polymer particles in the coating solution is preferably 1 to 70% by mass, more preferably 10 to 40% by mass. If the ratio of the hollow polymer particles is too low, sufficient heat insulation cannot be obtained, whereas if the ratio of the hollow polymer particles is too large, the adhesion force between the hollow polymer particles is reduced, and thereby sufficient film strength cannot be obtained, causing deterioration in abrasion resistance.

The heat insulation layer of the heat-sensitive transfer image-receiving sheet of the present invention is free of any resins that are not resistant to an organic solvent, except for the hollow polymer particles. Incorporation of the resin that is not resistant to an organic solvent (resin having a dye-dyeing affinity) in the heat insulation layer, is not preferable, in view of increase in loss of image definition after image transfer. It

is assumed that the color-edge definition loss increases by the reason that owing to the presence of both the resin having a dye-dyeing affinity and the hollow polymer particles in the heat insulation layer, a transferred dye that has dyed the receptor layer migrates through the heat insulation layer adjacent thereto with the lapse of time.

Herein, the term "the resin that is not resistant to an organic solvent" means a resin having solubility in an organic solvent (e.g., methyl ethyl ketone, ethyl acetate, benzene, toluene, xylene) of 1 mass % or more, preferably 0.5 mass % or more. For example, the above-mentioned latex polymer is included in the category of "the resin that is not resistant to an organic solvent".

The heat insulation layer preferably contains the above-mentioned water-soluble polymer. Preferable compounds of the water-soluble polymer to be used are the same as mentioned above.

An amount of the water-soluble polymer to be added in the heat insulation layer is preferably from 1 to 75 mass %, more preferably from 1 to 50 mass %, to the entire heat insulation layer.

The heat insulation layer preferably contains a gelatin. The amount of the gelatin in the coating solution for the heat insulation layer is preferably 0.5 to 14% by mass, and particularly preferably 1 to 6% by mass. Also, the coating amount of the above hollow polymer particles in the heat insulation layer is preferably 1 to 100 g/m<sup>2</sup>, and more preferably 5 to 20 g/m<sup>2</sup>.

The heat insulation layer preferably contains a crosslinking agent (which is a compound capable of crosslinking, for example, a water-soluble polymer). A part or all of the water-soluble polymer that is contained in the heat insulation layer has been preferably cross-linked with the crosslinking agent. Preferable compounds as well as a preferable amount of the crosslinking agent to be used are the same as mentioned above.

A preferred ratio of a cross-linked water-soluble polymer in the heat insulation layer varies depending on the kind of the crosslinking agent to be used, but the water-soluble polymer in the heat insulation layer is crosslinked by preferably 0.1 to 20 mass %, more preferably 1 to 10 mass %, based on the entire water-soluble polymer.

A thickness of the heat insulation layer containing the hollow polymer particles is preferably from 5 to 50  $\mu\text{m}$ , more preferably from 5 to 40  $\mu\text{m}$ .

A void ratio (porosity ratio) of the heat insulation layer, which is calculated from the thickness of the heat insulation layer containing hollow polymer particles and the solid-matter coating amount of the heat insulation layer including the hollow polymer particles, is preferably 10 to 70%, and more preferably 15 to 60%. When the void ratio in the heat insulation layer is too low, sufficient heat insulation property cannot be obtained. When the void ratio is too large, the binding force among hollow polymer particles deteriorates, and thus sufficient film strength cannot be obtained, and abrasion resistance deteriorates.

The void ratio of the heat insulation layer as referred to herein is a value V calculated according to formula (b).

$$V = 1 - L / \sum g_i \cdot d_i$$

Formula (b)

In formula (b), L represents the thickness of the heat-insulating layer;  $g_i$  represents the coating amount of a particular material i in terms of solid matter for the heat-insulating layer; and  $d_i$  represents the specific density of the particular material i. When  $d_i$  represents the specific density of the hollow polymer particles,  $d_i$  is the specific density of the wall material of hollow polymer particles.

## (Undercoat Layer)

An undercoat layer may be formed between the receptor layer and the heat insulation layer. As the undercoat layer, for example, at least one of a white background controlling layer, a charge controlling layer, an adhesive layer, and a primer layer is formed. These layers may be formed in the same manner as those described in, for example, each specification of Japanese Patent Nos. 3585599 and 2925244.

## (Support)

In the present invention, a waterproof support is preferably used as the support. The use of the waterproof support makes it possible to prevent the support from absorbing moisture, whereby a fluctuation in the performance of the receptor layer with the lapse of time can be prevented. As the waterproof support, for example, coated paper or laminate paper may be used.

## —Coated Paper—

The coated paper is paper obtained by coating a sheet, such as base paper, with various resins, latex rubbers, or high-molecular materials, on one side or both sides of the sheet, wherein the coating amount differs depending on its use. Examples of such coated paper include art paper, cast coated paper, and Yankee paper.

It is proper to use a thermoplastic resin as the resin to be applied to the surface(s) of the base paper and the like. As such a thermoplastic resin, for example, the following thermoplastic resins (A) to (H) may be exemplified.

(A) Polyolefin resins, such as polyethylene resin and polypropylene resin; copolymer resins composed of an olefin, such as ethylene or propylene, and another vinyl monomer; and acrylic resins.

(B) Thermoplastic resins having an ester linkage: for example, polyester resins obtained by condensation of a dicarboxylic acid component (such a dicarboxylic acid component may be substituted with a sulfonic acid group, a carboxyl group, or the like) and an alcohol component (such an alcohol component may be substituted with a hydroxyl group, or the like); polyacrylate resins or polymethacrylate resins, such as polymethyl methacrylate, polybutyl methacrylate, polymethyl acrylate, polybutyl acrylate, or the like; polycarbonate resins, polyvinyl acetate resins, styrene acrylate resins, styrene/methacrylate copolymer resins, vinyltoluene acrylate resins, or the like.

Concrete examples of them are those described in JP-A-59-101395, JP-A-63-7971, JP-A-63-7972, JP-A-63-7973, and JP-A-60-294862.

Commercially available thermoplastic resins usable herein are, for example, Vylon 290, Vylon 200, Vylon 280, Vylon 300, Vylon 103, Vylon GK-140, and Vylon GK-130 (products of Toyobo Co., Ltd.); Tafton NE-382, Tafton U-5, ATR-2009, and ATR-2010 (products of Kao Corporation); Elitel UE 3500, UE 3210, XA-8153, KZA-7049, and KZA-1449 (products of Unitika Ltd.); and Polyester TP-220, and R-188 (products of The Nippon Synthetic Chemical Industry Co., Ltd.); and thermoplastic resins in the Hyros series from Seiko Chemical Industries Co., Ltd., and the like (all of these names are trade names).

(C) Polyurethane resins, etc.

(D) Polyamide resins, urea resins, etc.

(E) Polysulfone resins, etc.

(F) Polyvinyl chloride resins, polyvinylidene chloride resins, vinyl chloride/vinyl acetate copolymer resins, vinyl chloride/vinyl propionate copolymer resins, etc.

(G) Polyol resins, such as polyvinyl butyral; and cellulose resins, such as ethyl cellulose resin and cellulose acetate resin.

(H) Polycaprolactone resins, styrene/maleic anhydride resins, polyacrylonitrile resins, polyether resins, epoxy resins, and phenolic resins.

The thermoplastic resins may be used either alone or in combination of two or more.

The thermoplastic resin may contain a whitener, a conductive agent, a filler, a pigment or dye including, for example, titanium oxide, ultramarine blue, and carbon black; or the like, if necessary.

## 10 —Laminated Paper—

The laminated paper is a paper which is formed by laminating various kinds of resin, rubber, polymer sheets or films on a sheet, such as a base paper or the like. Specific examples of the materials useable for the lamination include polyolefins, polyvinyl chlorides, polyethylene terephthalates, polystyrenes, polymethacrylates, polycarbonates, polyimides, and triacetylcelluloses. These resins may be used alone, or in combination of two or more.

Generally, the polyolefins are prepared by using a low-density polyethylene in many cases. For improving the thermal resistance of the support, it is preferred to use, for example, a polypropylene, a blend of a polypropylene and a polyethylene, a high-density polyethylene, or a blend of a high-density polyethylene and a low-density polyethylene. 20 From the viewpoint of costs and suitableness for the laminate, it is particularly preferred to use the blend of a high-density polyethylene and a low-density polyethylene.

The blend of a high-density polyethylene and a low-density polyethylene is used in a blend ratio (a mass ratio) of, for example, 1/9 to 9/1, preferably 2/8 to 8/2, and more preferably 3/7 to 7/3. When the thermoplastic resin layer is formed on the both surfaces of the support, the back side of the support is preferably formed using, for example, the high-density polyethylene or the blend of a high-density polyethylene and a low-density polyethylene. The molecular weight of the polyethylenes is not particularly limited. Preferably, both of the high-density polyethylene and the low-density polyethylene have a melt index of 1.0 to 40 g/10 minute and a high extrudability.

40 The sheet or film may be subjected to a treatment to impart white reflection thereto. As a method of such a treatment, for example, a method of incorporating a pigment, such as titanium oxide, into the sheet or film, can be mentioned.

The thickness of the support is preferably from 25  $\mu$ m to 300  $\mu$ m, more preferably from 50  $\mu$ m to 260  $\mu$ m, and further preferably from 75  $\mu$ m to 220  $\mu$ m. The support can have any rigidity according to the purpose. When it is used as a support for electrophotographic image-receiving sheet of photographic image quality, the rigidity thereof is preferably near to that in a support for use in color silver halide photography. (Curling Control Layer)

50 When the support is exposed as it is, there is the case where the heat-sensitive transfer image-receiving sheet is made to curl by moisture and/or temperature in the environment. It is therefore preferable to form a curling control layer on the backside of the support. The curling control layer not only prevents the image-receiving sheet from curling but also has a water-proof function. For the curling control layer, a polyethylene laminate, a polypropylene laminate or the like is used. Specifically, the curling control layer may be formed in a manner similar to those described in, for example, JP-A-61-110135 and JP-A-6-202295.

(Writing Layer and Charge Controlling Layer)

55 For the writing layer and the charge control layer, an inorganic oxide colloid, an ionic polymer, or the like may be used. As the antistatic agent, use may be made of any antistatic agent including a cationic antistatic agent, such as a quater-

35

nary ammonium salt and a polyamine derivative, an anionic antistatic agent, such as an alkyl phosphate, and a nonionic antistatic agent, such as a fatty acid ester. Specifically, the writing layer and the charge control layer may be formed in a manner similar to those described, for example, in the specification of Japanese Patent No. 3585585.

In the present invention, the above-described resin that is not resistant to an organic solvent or the water-soluble polymer used in the image-receiving sheet, is preferably in the form of an aqueous (water-based) dispersion.

The method of producing the heat-sensitive transfer image-receiving sheet of the present invention is explained below.

The heat-sensitive transfer image-receiving sheet of the present invention can be preferably formed, by applying at least one receptor layer, an intermediate layer, and at least one heat-insulating layer, on a support, through simultaneous multi-layer coating.

It is known that in the case of producing an image-receiving sheet composed of plural layers having different functions from each other (for example, an air cell layer, a heat insulation layer, an intermediate layer, and a receptor layer) on a support, it may be produced by applying each layer successively one by one, or by overlapping the layers each already coated on a support or substrate, as shown in, for example, JP-A-2004-106283, JP-A-2004-181888 and JP-A-2004-345267. It has been known in photographic industries, on the other hand, that productivity can be greatly improved, for example, by providing plural layers through simultaneous multi-layer coating. For example, there are known methods, such as the so-called slide coating (a slide coating method) and curtain coating (a curtain coating method), as described in, for example, U.S. Pat. Nos. 2,761,791, 2,681,234, 3,508, 947, 4,457,256 and 3,993,019; JP-A-63-54975, JP-A-61-278848, JP-A-55-86557, JP-A-52-31727, JP-A-55-142565, JP-A-50-43140, JP-A-63-80872, JP-A-54-54020, JP-A-5-104061, JP-A-5-127305, and JP-B-49-7050; by Edgar B. Gutoff, et al., "Coating and Drying Defects: Troubleshooting Operating Problems", John Wiley & Sons Company, 1995, pp. 101-103.

In the present invention, the productivity is greatly improved and at the same time image defects can be remarkably reduced, by using the above simultaneous multilayer coating for the production of an image-receiving sheet having a multilayer structure.

The plural layers in the present invention are structured using resins as its major components. Coating solutions forming each layer are preferably water-dispersible latexes. The solid content by mass of the resin put in a latex state in each layer coating solution is preferably in a range from 5 to 80% and particularly preferably 20 to 60%. The average particle size of the resin contained in the above water-dispersed latex is preferably 5  $\mu\text{m}$  or less and particularly preferably 1  $\mu\text{m}$  or less. The above water-dispersed latex may contain a known additive, such as a surfactant, a dispersant, and a binder resin, according to the need.

In the present invention, it is preferred that a laminate composed of plural layers be formed on a support and solidified just after the forming, according to the method described in U.S. Pat. No. 2,761,791. For example, in the case of solidifying a multilayer structure by using a resin, it is preferable to raise the temperature immediately after the plural layers are formed on the support. Also, in the case where a binder (e.g., a gelatin) to be gelled at lower temperatures is contained, there is the case where it is preferable to drop the temperature immediately after the plural layers are formed on the support.

In the present invention, the coating amount of a coating solution per one layer constituting the multilayer is preferably

36

in a range from 1  $\text{g}/\text{m}^2$  to 500  $\text{g}/\text{m}^2$ . The number of layers in the multilayer structure may be arbitrarily selected from a number of 2 or more. The receptor layer is preferably disposed as a layer most apart from the support.

5 A heat-sensitive transfer sheet (ink sheet) to be used in combination with the heat-sensitive transfer image-receiving sheet of the present invention as mentioned above at the time of formation of heat transfer image, is preferably a sheet having on a support a dye layer containing a diffusion-transferring dye, and any ink sheet can be used as the sheet. As a means for providing heat energy in the thermal transfer, any of the conventionally known providing means may be used. For example, application of a heat energy of about 5 to 100  $\text{mJ}/\text{mm}^2$  by controlling recording time in a recording device, 10 such as a thermal printer (trade name: Video Printer VY-100, manufactured by Hitachi, Ltd.), can sufficiently attain the expected result.

Also, the heat-sensitive transfer image-receiving sheet of the present invention may be used in various applications 20 enabling thermal transfer recording, such as heat-sensitive transfer image-receiving sheets in a form of thin sheets (cut sheets) or rolls; cards; and transmittable type manuscript-making sheets, by optionally selecting the type of support.

The present invention can be applied to a printer, a copying machine, and the like, each of which uses a heat-sensitive 25 transfer recording system.

The present invention can provide a heat-sensitive transfer image-receiving sheet which exhibits high productivity, 30 excellent in safety and environmental friendliness, which gives high sensitivity and high density, and which is good in releasing property from an ink sheet (no adhesion of the image-receiving sheet remains on the ink sheet). Further, the present invention can also provide a heat-sensitive transfer image-receiving sheet excellent in long-term preservability. 35 Furthermore, according to the present invention, it is possible to provide a heat-sensitive transfer image-receiving sheet, which is high in productivity and in environmental friendliness and safety, has high sensitivity, and can form a high-quality image high in density and excellent in long-term 40 preservability.

The present invention will be described in more detail based on the following examples, but the invention is not intended to be limited thereto.

## EXAMPLES

In the following examples, the terms "part" and "%" are values by mass, unless otherwise specified.

(Preparation of Ink Sheet)

50 A polyester film 6.0  $\mu\text{m}$  in thickness (trade name: Lumirror, manufactured by Toray Industries, Inc.) was used as a substrate film. A heat-resistant slip layer (thickness: 1  $\mu\text{m}$ ) was formed on the back side of the film, and the following yellow, magenta, and cyan compositions were respectively 55 applied as a monochromatic layer (coating amount: 1  $\text{g}/\text{m}^2$  after drying) on the front side.

### Yellow composition

|                                                                                             |                   |
|---------------------------------------------------------------------------------------------|-------------------|
| Dye (trade name: Macrolex Yellow 6G, manufactured by Byer)                                  | 5.5 parts by mass |
| Polyvinylbutyral resin (trade name: ESLEC BX-1, manufactured by Sekisui Chemical Co., Ltd.) | 4.5 parts by mass |
| Methyl ethyl ketone/toluene (1/1, at mass ratio)                                            | 90 parts by mass  |

| Magenta composition                                                                         |                   |
|---------------------------------------------------------------------------------------------|-------------------|
| Magenta dye (Disperse Red 60)                                                               | 5.5 parts by mass |
| Polyvinylbutyral resin (trade name: ESLEC BX-1, manufactured by Sekisui Chemical Co., Ltd.) | 4.5 parts by mass |
| Methyl ethyl ketone/toluene (1/1, at mass ratio)                                            | 90 parts by mass  |
| Cyan composition                                                                            |                   |
| Cyan dye (Solvent Blue 63)                                                                  | 5.5 parts by mass |
| Polyvinylbutyral resin (trade name: ESLEC BX-1, manufactured by Sekisui Chemical Co., Ltd.) | 4.5 parts by mass |
| Methyl ethyl ketone/toluene (1/1, at mass ratio)                                            | 90 parts by mass  |

A pulp slurry was prepared from 50 parts by mass of hardwood kraft pulp (LBKP) of acacia origin and 50 parts by mass of hardwood kraft pulp (LBKP) of aspen origin, by beating these pulps by means of a disk refiner until Canadian standard freeness reached to 300 ml.

To the pulp slurry thus prepared were added, on a pulp basis, 1.3 mass % of modified cationic starch (CAT0304L, trade name, manufactured by Nippon NSC), 0.15 mass % of anionic polyacrylamide (DA4104, trade name, manufactured by Seiko PMC Corporation), 0.29 mass % of an alkylketene dimer (SIZEPINE K, trade name, manufactured by Arakawa Chemical Industries, Ltd.), 0.29 mass % of epoxidized behenic acid amide, and 0.32 mass % of polyamide polyamine epichlorohydrin (ARAFIX 100, trade name, manufactured by Arakawa Chemical Industries, Ltd.), and thereafter 0.12 mass % of a defoaming agent was further added.

The resulting pulp slurry was made into paper by use of a fourdrinier paper machine. In a process of drying in which the felt side of web was pressed against a drum dryer cylinder via a dryer canvas, the web thus formed was dried under a condition that the tensile strength of the dryer canvas was adjusted to 1.6 kg/cm. Then, each side of the raw paper thus made was coated with 1 g/m<sup>2</sup> of polyvinyl alcohol (KL-118, trade name, manufactured by Kuraray Co., Ltd.) with a size press, then, dried and further subjected to calendering treatment. Therein, the papermaking was performed so that the raw paper had a grammage (basis weight) of 157 g/m<sup>2</sup>, and the raw paper (base paper) having a thickness of 160 µm was obtained.

The wire side (back side) of the base paper obtained was subjected to corona discharge treatment, and thereto a resin composition, in which a high-density polyethylene having an MFR (which stands for a melt flow rate, and hereinafter has the same meaning) of 16.0 g/10 min and a density of 0.96 g/cm<sup>3</sup> (containing 250 ppm of hydrotalcite (DHT-4A (trade name), manufactured by Kyowa Chemical Industry Co., Ltd.) and 200 ppm of a secondary antioxidant (tris(2,4-di-t-butylphenyl)phosphite, Irugaphos 168 (trade name), manufactured by Ciba Specialty Chemicals)) and a low-density polyethylene having an MFR of 4.0 g/10 min and a density of 0.93 g/cm<sup>3</sup> were mixed at a ratio of 75 to 25 by mass, was applied so as to have a thickness of 21 g/m<sup>2</sup>, by means of a melt extruder, thereby forming a thermoplastic resin layer with a mat surface. (The side to which this thermoplastic resin layer was provided is hereinafter referred to as "back side"). The

thermoplastic resin layer at the back side was further subjected to corona discharge treatment, and then coated with a dispersion prepared by dispersing into water a 1:2 mixture (by mass) of aluminum oxide (ALUMINASOL 100, trade name, manufactured by Nissan Chemical Industries, Ltd.) and silicon dioxide (SNOWTEX O, trade name, manufactured by Nissan Chemical Industries, Ltd.), as an antistatic agent, so that the coating had a dry mass of 0.2 g/m<sup>2</sup>. Subsequently, the front surface (front side) of the base paper was subjected to corona discharge treatment, and then coated with 27 g/m<sup>2</sup> of a low-density polyethylene having an MFR of 4.0 g/10 min and a density of 0.93 g/m<sup>3</sup> and containing 10 mass % of titanium oxide, by means of a melt extruder, thereby forming a thermoplastic resin layer with a specular surface.

(Preparation of Emulsified Dispersion A)

An emulsified dispersion A was prepared in the following manner. An antioxidant (EB-9) was dissolved in a mixture of 42 g of a high-boiling solvent (Solv-5) and 20 ml of ethyl acetate, and the resulting solution was emulsified and dispersed in 250 g of a 20 mass % aqueous gelatin solution containing 1 g of sodium dodecylbenzenesulfonate by means of a high-speed stirring emulsification machine (dissolver). Thereto, water was added to prepare 380 g of an emulsified dispersion A.

Therein, the addition amount of the antioxidant agent (EB-9) was adjusted so that the antioxidant agent would be contained in an amount of 30 mol % in the emulsified dispersion A.

Example 1

Preparation of Latex Polymer 1

After the atmosphere in a polymerization vessel equipped with a stirrer, a condenser, a thermometer, and an inlet for introduction of nitrogen gas, was thoroughly replaced with N<sub>2</sub>, 1,150 g of deionized water, 100 g of methyl acrylate, and 30 g of sodium dodecylbenzenesulfonate were placed in the vessel, the pressure inside the polymerization vessel was reduced, and then 900 parts by mass of vinyl chloride was further placed therein. After the temperature inside the polymerization vessel was raised to 60° C., 50 parts by mass of a 1% aqueous solution of ammonium persulfate was introduced under pressure to initiate polymerization reaction, and the reaction was continued for 16 hours as the inside temperature was kept at 60° C., to attain completion of the polymerization. Thereafter, the reaction liquid was cooled to 30° C., and adjusted to the pH within a range of from 7 to 8 by use of 25% aqueous ammonia. Thus, a latex polymer 1 (emulsion) was prepared, and this emulsion was applied to a dry glass plate, and then only the polymer component from the resultant coating was extracted with chloroform. This extract was analyzed by <sup>1</sup>H-NMR measurement, and the vinyl chloride/methyl acrylate ratio was determined to be 90:10 as the composition of the above-prepared latex polymer 1 (emulsion). (Preparation of Latex Polymers 2 to 9)

Latex polymers 2 to 9 were prepared in the same manner as the latex polymer 1, except that the amounts of vinyl chloride used and the numbers of carbon atoms in alcohol-derived moieties of acrylic acid esters used were changed to those shown in Table 1, respectively. Hereinafter, the alcohol-derived moiety of an acrylic acid ester is referred to as "alkyl moiety", and the number of carbon atoms contained therein is referred to as "alkyl carbon number".

TABLE 1

| Polymer composition |                     |                                                         |
|---------------------|---------------------|---------------------------------------------------------|
| Latex polymer       | Vinyl chloride unit | Acrylate unit<br>(Alkyl carbon number:<br>Alkyl moiety) |
| 1                   | 90                  | 10 (1)                                                  |
| 2                   | 90                  | 10 (2)                                                  |
| 3                   | 90                  | 10 (3)                                                  |
| 4                   | 90                  | 10 (4)                                                  |
| 5                   | 90                  | 10 (6)                                                  |
| 6                   | 90                  | 10 (8)                                                  |
| 7                   | 90                  | 10 (12)                                                 |
| 8                   | 30                  | 70 (2)                                                  |
| 9                   | 30                  | 70 (4)                                                  |

(Preparation of Heat-Sensitive Transfer Image-Receiving Sheet 101 (This Invention))

A sample was prepared by simultaneous multi-layer coating, so as to form a multiple-layer structure, on the support prepared in the foregoing manner, having a subbing layer, a heat insulation layer, and a receptor layer, in increasing order of distance from the support. Compositions and application amounts of the coating solutions used herein are shown below.

| Coating solution for subbing layer<br>(Composition)                             |                  |
|---------------------------------------------------------------------------------|------------------|
| Latex styrene/butadiene (SR103 (trade name), manufactured by Nippon A & L Inc.) | 93 parts by mass |
| 8.7% Aqueous solution of polyvinyl alcohol (PVA)                                | 57 parts by mass |
| NaOH for adjusting pH to 8<br>(Coating amount) 21 ml/m <sup>2</sup>             |                  |

| Coating solution for heat insulation layer<br>(Composition)                            |                  |
|----------------------------------------------------------------------------------------|------------------|
| Hollow latex polymer particles (MH5055 (trade name), manufactured by Zeon Corporation) | 38 parts by mass |
| 16% Gelatin aqueous solution                                                           | 26 parts by mass |
| Water                                                                                  | 4 parts by mass  |
| NaOH for adjusting pH to 8<br>(Coating amount) 45 ml/m <sup>2</sup>                    |                  |

| Coating solution for receptor layer<br>(Composition)                                    |                  |
|-----------------------------------------------------------------------------------------|------------------|
| Latex polymer 1 prepared (solid content 40% by mass)                                    | 50 parts by mass |
| 10% Gelatin aqueous solution                                                            | 10 parts by mass |
| Emulsified dispersion A prepared in the above                                           | 13 parts by mass |
| Microcrystalline wax (EMUSTAR-42X (trade name), manufactured by Nippon Seiro Co., Ltd.) | 7 parts by mass  |
| Water                                                                                   | 35 parts by mass |
| NaOH for adjusting pH to 8<br>(Coating amount) 18 ml/m <sup>2</sup>                     |                  |

Immediately before coating, a compound X (cross-linking agent) illustrated below was added to the foregoing receptor layer coating solution. The amount of the compound X added

was adjusted to 3 mass % based on the total mass of gelatin in the heat-insulating layer and the receptor layer.



(Preparation of Heat-Sensitive Transfer Image-Receiving Sheets 102 to 109)

15 Heat-sensitive transfer image-receiving sheets 102 to 109 were prepared in the same manner as the heat-sensitive transfer image-receiving sheet 101, except that the latex polymer 1 used in the image-receiving layer was replaced with any of the latex polymers 2 to 9 prepared in this example, respectively. Incidentally, the latex polymers were each added in the same amount on a solids basis.

20 (Preparation of Heat-Sensitive Transfer Image-Receiving Sheet 110 (Comparative Example))

25 Heat-sensitive transfer image-receiving sheet 110 was prepared in the same manner as the heat-sensitive transfer image-receiving sheet 101, except that the latex polymer 1 used in the image-receiving layer was replaced with a commercially available latex polymer (water-dispersible polyester: MD-1200, trade name, manufactured by TOYOB0 Co., Ltd.).

30 (Image Formation)

35 The ink sheet and any of the heat-sensitive transfer image-receiving sheets 101 to 110 were each worked so as to become loadable, and a printed output was produced on each combination of the ink sheet and any of the image-receiving sheets, in a high-speed print mode, by use of a sublimation-type thermal transfer printer ASK2000 (trade name, manufactured by FUJIFILM Corporation). More specifically, the black image (black solid image) of the maximum density on the entire face was used as an output image, and the output image was produced in succession on 20 pieces of each image-receiving sheet. Herein, the time interval between ejection of one printed piece and ejection of the next one was 8 seconds.

40 (Image Evaluation)

45 (1) Evaluation of Dmax

50 The visual density of the black solid image obtained in the above condition was measured by Photographic Densitometer (trade name, manufactured by X-Rite Incorporated).

(2) Evaluation of Releasing Property (Adhesive Property)

55 For evaluation of releasing property of the image-receiving sheet from the ink sheet, the black image (black solid image) of the maximum density on the entire face was output, on each image-receiving sheet in accordance with the foregoing method, and the surface of the obtained outputs were observed to evaluate the extent of streaked unevenness (sticking) on the surface thereof. At the same time, noises caused by this processing were caught and their volume was evaluated.

TABLE 2

| Sample No.<br>(Remarks)         | Latex composition              |          |                        | Evaluation of properties |                     |          |                         |
|---------------------------------|--------------------------------|----------|------------------------|--------------------------|---------------------|----------|-------------------------|
|                                 | Vinyl<br>chloride              | Acrylate | Alkyl carbon<br>number | Alkyl<br>moiety          | Transfer<br>density | Sticking | Ink sheet<br>peel noise |
| 101 (This<br>invention)         | 90                             | 10       | 1                      | Methyl                   | 2.02                | ◎        | ○                       |
| 102 (This<br>invention)         | 90                             | 10       | 2                      | Ethyl                    | 2.06                | ◎        | ◎                       |
| 103 (This<br>invention)         | 90                             | 10       | 3                      | Propyl                   | 2.08                | ○        | ○                       |
| 104 (This<br>invention)         | 90                             | 10       | 4                      | Butyl                    | 2.08                | ◎        | ◎                       |
| 105 (This<br>invention)         | 90                             | 10       | 6                      | Hexyl                    | 2.04                | ○        | Δ                       |
| 106 (This<br>invention)         | 90                             | 10       | 8                      | 2-Ethyl-<br>hexyl        | 2.09                | ○        | ○                       |
| 107 (This<br>invention)         | 90                             | 10       | 12                     | Dodecyl                  | 2.00                | Δ        | Δ                       |
| 108<br>(Comparative<br>example) | 30                             | 70       | 2                      | Ethyl                    | 1.65                | X        | X                       |
| 109<br>(Comparative<br>example) | 30                             | 70       | 4                      | Butyl                    | 1.57                | X        | X                       |
| 110<br>(Comparative<br>example) | MD1200<br>(Commercial product) |          |                        | 1.75                     | Δ                   | X        |                         |

These evaluation results were ranked as shown below, and the results are shown in Table 2.

Evaluation rank

◎: Better results than the level for ○ were obtained.

○: Good results were obtained without any problems.

Δ: Results obtained showed tendencies to deteriorate, but they were still on an acceptable level.

X: Result obtained had problems, so that they were on a practically unacceptable level.

By making comparisons among the Samples 101 to 110 (the Samples 101 to 107 according to the present invention versus the Samples 108 to 110 for comparison), it can be seen that satisfactory properties (i.e. transfer density, sticking, and ink-sheet peel noise) were exhibited by any of the vinyl chloride/acrylic acid ester copolymers containing vinyl chloride in a proportion of 50 mass % or more, according to the present invention.

In addition, comparisons among the Samples 101 to 107 indicate that, when the vinyl chloride/acrylate ratio was 9/1, the performance (i.e. transfer density, sticking, and ink-sheet peel noise) varied depending on the number of carbons in the alkyl group/moiety of the acrylate contained, and the cases where the number of alkyl carbons in the acrylate was from 1 to 8 exhibited especially satisfactory performance. Moreover, it can be found that, when the vinyl chloride/acrylate ratio is 9/1, those preferred as an alkyl moiety of the acrylate are methyl, ethyl, propyl, butyl, 2-ethylhexyl, and hexyl, the more preferred are methyl, ethyl, propyl, butyl, and 2-ethylhexyl, and the most preferred are ethyl and butyl.

### Example 2

#### Preparation of Latex Polymers 11 to 16

Latex polymers 11 to 16 were prepared in the same manner as the latex polymer 1, except that the amounts of vinyl chloride used and the alkyl carbon numbers and amounts of acrylic acid esters used were changed to those shown in Table 3, respectively.

TABLE 3

| Latex polymer | Vinyl chloride/acrylate ratio |                                               |
|---------------|-------------------------------|-----------------------------------------------|
|               | Vinyl chloride unit           | Alkyl carbon number 1<br>Methyl acrylate unit |
| 11            | 95                            | 5                                             |
| 12            | 80                            | 20                                            |
| 13            | 70                            | 30                                            |
| 14            | 60                            | 40                                            |
| 15            | 40                            | 60                                            |
| 16            | 30                            | 70                                            |

(Preparation of Heat-Sensitive Transfer Image-Receiving Sheets 111 to 116)

Heat-sensitive transfer image-receiving sheets 111 to 116 were prepared in the same manner as the heat-sensitive transfer image-receiving sheet 101, except that the latex polymer 1 used in the image-receiving layer was replaced with any of the latex polymers 11 to 16 prepared in this example, respectively. Incidentally, the latex polymers were each added in the same amount on a solids basis.

The same tests as in Example 1 were conducted on each of the thus-prepared heat-sensitive transfer image-receiving sheets 111 to 116. Results obtained are shown in Table 4.

TABLE 4

| Sample No.<br>(Remarks) | Latex composition |                    | Evaluation of properties |          |                         |
|-------------------------|-------------------|--------------------|--------------------------|----------|-------------------------|
|                         | Vinyl<br>Chloride | Methyl<br>acrylate | Transfer<br>density      | Sticking | Ink sheet<br>peel noise |
| 111 (This<br>invention) | 95                | 5                  | 1.91                     | ◎        | ○                       |
| 112 (This<br>invention) | 80                | 20                 | 2.02                     | ◎        | ○                       |

TABLE 4-continued

| Sample No.<br>(Remarks)         | Latex composition |                    | Evaluation of properties |          |                         |
|---------------------------------|-------------------|--------------------|--------------------------|----------|-------------------------|
|                                 | Vinyl<br>Chloride | Methyl<br>acrylate | Transfer<br>density      | Sticking | Ink sheet<br>peel noise |
| 113 (This<br>invention)         | 70                | 30                 | 2.05                     | ◎        | ○                       |
| 114 (This<br>invention)         | 60                | 40                 | 2.05                     | ○        | ○                       |
| 115<br>(Comparative<br>example) | 40                | 60                 | 1.70                     | Δ        | X                       |
| 116<br>(Comparative<br>example) | 30                | 70                 | 1.65                     | X        | X                       |

From comparisons among Samples 111 to 116, it can be seen that, when the alkyl carbon number of acrylic acid ester was 1, Samples 111 to 114 having their respective vinyl chloride/acrylic acid ester ratios in the range of 97/3 to 55/45 exhibited better performance. Of these ratios, in the case of methyl acrylate, the vinyl chloride/methyl acrylate ratios in the vicinity of 75/25 contributed the best performance.

## Example 3

## Preparation of Latex Polymers 21 to 26

Latex polymers 21 to 26 were prepared in the same manner as the latex polymer 1, except that the amounts of vinyl chloride used and the alkyl carbon numbers and amounts of acrylic acid esters used were changed to those shown in Table 5, respectively.

TABLE 5

| Latex polymer | Ratio of (vinyl chloride/acrylate) |                                              |
|---------------|------------------------------------|----------------------------------------------|
|               | Vinyl chloride unit                | Alkyl carbon number 2<br>Ethyl acrylate unit |
| 21            | 95                                 | 5                                            |
| 22            | 90                                 | 10                                           |
| 23            | 80                                 | 20                                           |
| 24            | 70                                 | 30                                           |
| 25            | 40                                 | 60                                           |
| 26            | 30                                 | 70                                           |

## (Preparation of Heat-Sensitive Transfer Image-Receiving Sheets 121 to 126)

Heat-sensitive transfer image-receiving sheets 121 to 126 were prepared in the same manner as the heat-sensitive transfer image-receiving sheet 101, except that the latex polymer 1 used in the image-receiving layer was replaced with any of the latex polymers 21 to 26 prepared in this example, respectively. Incidentally, the latex polymers were each added in the same amount on a solids basis.

The same tests as in Example 1 were prepared on each of the thus-prepared heat-sensitive transfer image-receiving sheets 121 to 126. Results obtained are shown in Table 6.

TABLE 6

| Sample No.<br>(Remarks) | Latex composition |                   | Evaluation of properties |          |                         |
|-------------------------|-------------------|-------------------|--------------------------|----------|-------------------------|
|                         | Vinyl<br>chloride | Ethyl<br>acrylate | Transfer<br>density      | Sticking | Ink sheet<br>peel noise |
| 121 (This<br>invention) | 95                | 5                 | 1.92                     | ◎        | ◎                       |

TABLE 6-continued

| Sample No.<br>(Remarks)         | Latex composition |                   | Evaluation of properties |          |                         |
|---------------------------------|-------------------|-------------------|--------------------------|----------|-------------------------|
|                                 | Vinyl<br>chloride | Ethyl<br>acrylate | Transfer<br>density      | Sticking | Ink sheet<br>peel noise |
| 122 (This<br>invention)         | 90                | 10                | 2.06                     | ◎        | ◎                       |
| 123 (This<br>invention)         | 80                | 20                | 2.08                     | ◎        | ○                       |
| 124 (This<br>invention)         | 70                | 30                | 2.02                     | ○        | Δ                       |
| 125<br>(Comparative<br>example) | 40                | 60                | 1.62                     | X        | X                       |
| 126<br>(Comparative<br>example) | 30                | 70                | 1.57                     | X        | X                       |

From comparisons among Samples 121 to 126, it can be seen that, when the alkyl carbon number of acrylic acid esters was 2, Samples 121 to 124 having their respective vinyl chloride/acrylic acid ester ratios in the range of 95/5 to 55/45 exhibited better performance. Of these ratios, in the case of ethyl acrylate, the vinyl chloride/ethyl acrylate ratios in the vicinity of 80/20 contributed the best performance.

## Example 4

## Preparation of Latex Polymers 31 to 36

Latex polymers 31 to 36 were prepared in the same manner as the latex polymer 1, except that the amounts of vinyl chloride used and the alkyl carbon numbers and amounts of acrylic acid esters used were changed to those shown in Table 7, respectively.

TABLE 7

| Latex polymer | Ratio of (vinyl acetate/acrylate) |                                              |
|---------------|-----------------------------------|----------------------------------------------|
|               | Vinyl chloride unit               | Alkyl carbon number 4<br>Butyl acrylate unit |
| 31            | 98                                | 2                                            |
| 32            | 95                                | 5                                            |
| 33            | 90                                | 10                                           |
| 34            | 80                                | 20                                           |
| 35            | 40                                | 60                                           |
| 36            | 30                                | 70                                           |

## (Preparation of Heat-Sensitive Transfer Image-Receiving Sheets 131 to 136)

Heat-sensitive transfer image-receiving sheets 131 to 136 were prepared in the same manner as the heat-sensitive transfer image-receiving sheet 101, except that the latex polymer 1 used in the image-receiving layer was replaced with any of the latex polymers 31 to 36 prepared in this example, respectively. Incidentally, the latex polymers were each added in the same amount on a solids basis.

The same tests as in Example 1 were conducted on each of the thus-prepared heat-sensitive transfer image-receiving sheets 131 to 136. Results obtained are shown in Table 8.

TABLE 8

| Sample No.<br>(Remarks)         | Latex composition |                   | Evaluation of properties |          |                         |
|---------------------------------|-------------------|-------------------|--------------------------|----------|-------------------------|
|                                 | Vinyl<br>chloride | Butyl<br>acrylate | Transfer<br>density      | Sticking | Ink sheet<br>peel noise |
| 131 (This<br>invention)         | 98                | 2                 | 1.90                     | ◎        | ○                       |
| 132 (This<br>invention)         | 95                | 5                 | 2.08                     | ◎        | ○                       |
| 133 (This<br>invention)         | 90                | 10                | 2.08                     | ◎        | ◎                       |
| 134 (This<br>invention)         | 80                | 20                | 2.11                     | ○        | ○                       |
| 135<br>(Comparative<br>example) | 40                | 60                | 1.70                     | X        | X                       |
| 136<br>(Comparative<br>example) | 30                | 70                | 1.56                     | X        | X                       |

From comparisons among Samples 131 to 136, it can be seen that, when the alkyl carbon number of acrylic acid ester was 4, Samples 131 to 134 having their respective vinyl chloride/acrylic acid ester ratios in the range of 98/2 to 70/30 exhibited better performance. Of these ratios, in the case of butyl acrylate, the vinyl chloride/butyl acrylate ratios in the vicinity of 90/10 contributed the best performance.

## Example 5

## Preparation of Latex Polymers 41 to 45

Latex polymers 41 to 45 were prepared in the same manner as the latex polymer 1, except that the amounts of vinyl chloride used and the alkyl carbon numbers and amounts of acrylic acid esters used were changed to those shown in Table 9, respectively.

TABLE 9

| Latex polymer | Vinyl chloride/acrylate ratio |                            | Alkyl carbon number 8<br>2-ethylhexyl acrylate unit |
|---------------|-------------------------------|----------------------------|-----------------------------------------------------|
|               | Vinyl chloride unit           | 2-ethylhexyl acrylate unit |                                                     |
| 41            | 97                            | 3                          |                                                     |
| 42            | 94                            | 6                          |                                                     |
| 43            | 85                            | 15                         |                                                     |
| 44            | 70                            | 30                         |                                                     |
| 45            | 40                            | 60                         |                                                     |

(Preparation of Heat-Sensitive Transfer Image-Receiving Sheets 141 to 145)

Heat-sensitive transfer image-receiving sheets 141 to 145 were prepared in the same manner as the heat-sensitive transfer image-receiving sheet 101, except that the latex polymer 1 used in the image-receiving layer was replaced with any of the latex polymers 41 to 45 prepared in this example, respectively. Incidentally, the latex polymers were each added in the same amount on a solids basis.

The same tests as in Example 1 were conducted on each of the thus-prepared heat-sensitive transfer image-receiving sheets 141 to 145. Results obtained are shown in Table 10.

TABLE 10

| Sample No.<br>(Remarks)         | Latex composition |                          | Evaluation of properties |          |                         |
|---------------------------------|-------------------|--------------------------|--------------------------|----------|-------------------------|
|                                 | Vinyl<br>chloride | 2-Ethylhexyl<br>acrylate | Transfer<br>density      | Sticking | Ink sheet<br>peel noise |
| 141 (This<br>invention)         | 97                | 3                        | 1.99                     | ◎        | ○                       |
| 142 (This<br>invention)         | 94                | 6                        | 2.09                     | ◎        | ○                       |
| 143 (This<br>invention)         | 85                | 15                       | 2.07                     | ◎        | ◎                       |
| 144 (This<br>invention)         | 70                | 30                       | 2.02                     | ○        | Δ                       |
| 145<br>(Comparative<br>example) | 40                | 60                       | 1.78                     | X        | X                       |

From comparisons among Samples 141 to 145, it can be seen that, when the alkyl carbon number of acrylic acid ester was 8, Samples 141 to 144 having their respective vinyl chloride/acrylic acid ester ratios in the range of 98/2 to 75/25 exhibited better performance. Of these ratios, in the case of 2-ethylhexyl acrylate, the vinyl chloride/2-ethylhexyl acrylate ratios in the vicinity of 85/15 to 90/10 contributed the best performance.

## Example 6

## Preparation of Latex Polymers 51 to 58

Latex polymers 51 to 58 were prepared in the same manner as the latex polymer 1, except that the amounts of vinyl chloride used and the alkyl carbon numbers and amounts of acrylic acid esters used were changed to those shown in Table 11, respectively.

TABLE 11

| Latex polymer | Vinyl chloride/acrylate ratio |                                               | Alkyl carbon number 3<br>Propyl acrylate unit |
|---------------|-------------------------------|-----------------------------------------------|-----------------------------------------------|
|               | Vinyl chloride unit           | Alkyl carbon number 3<br>Propyl acrylate unit |                                               |
| 51            | 90                            | 10                                            |                                               |
| 52            | 80                            | 20                                            |                                               |
| 53            | 60                            | 40                                            |                                               |
| 54            | 40                            | 60                                            |                                               |

  

| Latex polymer | Alkyl carbon number 6<br>Hexyl acrylate unit |                                              |
|---------------|----------------------------------------------|----------------------------------------------|
|               | Vinyl chloride unit                          | Alkyl carbon number 6<br>Hexyl acrylate unit |
| 55            | 90                                           | 10                                           |
| 56            | 80                                           | 20                                           |
| 57            | 60                                           | 40                                           |
| 58            | 40                                           | 60                                           |

(Preparation of Heat-Sensitive Transfer Image-Receiving Sheets 151 to 158)

Heat-sensitive transfer image-receiving sheets 151 to 158 were prepared in the same manner as the heat-sensitive transfer image-receiving sheet 101, except that the latex polymer 1 used in the image-receiving layer was replaced with any of the latex polymers 51 to 58 prepared in this example, respectively. Incidentally, the latex polymers were each added in the same amount on a solids basis.

The same tests as in Example 1 were conducted on each of the thus-prepared heat-sensitive transfer image-receiving sheets 151 to 158. Results obtained are shown in Table 12.

TABLE 12

| Sample No.<br>(Remarks)   | Latex composition |                 | Evaluation of properties |          |                      |
|---------------------------|-------------------|-----------------|--------------------------|----------|----------------------|
|                           | Vinyl chloride    | Propyl acrylate | Transfer density         | Sticking | Ink sheet peel noise |
| 151 (This invention)      | 90                | 10              | 2.08                     | ○        | ○                    |
| 152 (This invention)      | 80                | 20              | 2.09                     | ○        | ○                    |
| 153 (This invention)      | 60                | 40              | 1.94                     | ○        | △                    |
| 154 (Comparative example) | 40                | 60              | 1.64                     | X        | X                    |
| Sample No.<br>(Remarks)   | Vinyl chloride    | Hexyl acrylate  | Transfer density         | Sticking | Ink sheet peel noise |
| 155 (This invention)      | 90                | 10              | 2.04                     | ○        | ○                    |
| 156 (This invention)      | 80                | 20              | 2.03                     | ○        | ○                    |
| 157 (This invention)      | 60                | 40              | 1.83                     | ○        | △                    |
| 158 (Comparative example) | 40                | 60              | 1.72                     | X        | X                    |

From comparisons among the Samples 151 to 158, it can be seen that, when the alkyl carbon number in acrylic acid ester was respectively 3 or 6, Samples 151, 152, 153, 155, 156, and 157 meeting the vinyl chloride/acrylic acid ester ratio requirement as defined in the present invention fully achieved all of the performance covering transfer density, sticking, and ink-sheet peel noise.

From comparisons among Samples 151 to 154, it can be seen that, when the alkyl carbon number of acrylic acid ester was 3, Samples 151 to 152 having their respective vinyl chloride/acrylic acid ester ratios in the range of 95/5 to 65/35 exhibited better performance.

TABLE 13

| 5  | Ratio of (vinyl chloride/acrylate/vinyl acetate) |                     |                                |                    |
|----|--------------------------------------------------|---------------------|--------------------------------|--------------------|
|    | Latex polymer                                    | Vinyl chloride unit | Acrylate unit (Alkyl moiety)   | Vinyl acetate unit |
| 10 | 61                                               | 90                  | —                              | 10                 |
|    | 62                                               | 85                  | —                              | 15                 |
|    | 63                                               | 65                  | —                              | 35                 |
|    | 64                                               | 90                  | 5 (Butyl),<br>5 (Ethyl)        | —                  |
| 15 | 65                                               | 90                  | 5 (Butyl),<br>5 (2-Ethylhexyl) | —                  |
|    | 66                                               | 90                  | 5 (Butyl)                      | 5                  |
|    | 67                                               | 85                  | 5 (Ethyl)                      | 10                 |
|    | 68                                               | 40                  | 30 (Ethyl)                     | 30                 |

(Preparation of Heat-Sensitive Transfer Image-Receiving Sheets 161 to 168)

Heat-sensitive transfer image-receiving sheets 161 to 168 were prepared in the same manner as the heat-sensitive transfer image-receiving sheet 101, except that the latex polymer 1 used in the image-receiving layer was replaced with any of the latex polymers 61 to 68 prepared in this example, respectively. Incidentally, the latex polymers were each added in the same amount on a solids basis.

The same tests as in Example 1 were conducted on each of the thus-prepared heat-sensitive transfer image-receiving sheets 161 to 168. Results obtained are shown in Table 14.

TABLE 14

| Sample No.<br>(Remarks)   | Latex composition |          | Evaluation of properties |                  |                      |
|---------------------------|-------------------|----------|--------------------------|------------------|----------------------|
|                           | Vinyl chloride    | Acrylate | Vinyl acetate            | Transfer density | Ink sheet peel noise |
| 161 (This invention)      | 90                | —        | 10                       | 2.01             | ○ ○                  |
| 162 (This invention)      | 85                | —        | 15                       | 2.06             | ○ ○                  |
| 163 (This invention)      | 65                | —        | 35                       | 1.74             | ○ △                  |
| 164 (This invention)      | 90                | 5 and 5  | —                        | 2.03             | ○ ○                  |
| 165 (This invention)      | 90                | 5 and 5  | —                        | 2.05             | ○ ○                  |
| 166 (This invention)      | 90                | 5        | 5                        | 2.05             | ○ ○                  |
| 167 (This invention)      | 85                | 5        | 10                       | 2.05             | ○ ○                  |
| 168 (Comparative example) | 40                | 30       | 30                       | 1.54             | X X                  |

From comparisons among Samples 155 to 158, it can be seen that, when the alkyl carbon number of acrylic acid ester was 6, Samples 155 to 156 having their respective vinyl chloride/acrylic acid ester ratios in the range of 97/3 to 72/28 exhibited better performance.

### Example 7

#### Preparation of Latex Polymers 61 to 68

Latex polymers 61 to 68 were prepared in the same manner as the latex polymer 1, except that the amounts of vinyl chloride used and the amounts of vinyl acetate used instead of the acrylic acid ester were changed to those shown in Table 13, respectively.

From comparisons among Samples 161 to 168, it can be seen that Samples 161 to 163 having the vinyl chloride/vinyl acetate ratios of their respective latex polymers in the range specified by the present invention, Samples 164 and 165 composed of the vinyl chloride/acrylate/acrylate terpolymers according to the present invention, and Samples 166 and 167 composed of the vinyl chloride/acrylate/vinyl acetate terpolymers according to the present invention, each were excellent in the properties.

When image formation was carried out in the same manner as in the Examples 1 to 7, except that the heat-sensitive transfer image-receiving sheets used in the Examples 1 to 7 were changed to those prepared in this example, and that the printer used in the Examples 1 to 7 was changed to a sublimation-type thermal transfer printer CW01 (trade name,

manufactured by Citizen Co., Ltd.), the heat-sensitive transfer image-receiving sheets of the present invention achieved good results as in the case of the samples according to the present invention prepared in Examples 1 to 7.

#### Example 8

Latex polymers A to E were prepared in the same manner as the latex polymer 1 in Example 1, except that the acrylic acid ester to be copolymerized with the vinyl chloride monomer was changed to any of different acrylic acid esters shown in Table 15, respectively. More specifically, the latex polymers A to E were samples whose constituent polymers were adjusted to have their glass transition temperatures in the vicinity of 65° C. by polymerizing vinyl chloride together with any of the different acrylic acid esters, respectively, in copolymerization ratios different from one another.

Then, Samples 801 to 805 were prepared in the same manner as Sample 101, except that the latex polymer 1 was changed to any of the latex polymers A to E, respectively.

In addition, Sample 806 was prepared in the same manner as Sample 802, except that no gelatin was added to the receptor layer.

Moreover, Sample 807 was prepared in the same manner as Sample 802, except that the heat-insulating layer was not coated, and Sample 808 was prepared in the same manner as Sample 802, except that the successive coating was adopted in which the receptor layer was coated after the double-layer coating of the subbing layer and the heat-insulating layer was applied and then dried.

In addition, Sample 809 was prepared in the same manner as Sample 802, except that no gelatin was added to the heat insulation layer.

#### (Image Formation)

The ink sheet and any of the heat-sensitive transfer image-receiving sheet samples 801 to 809 were each worked so as to become loadable, and a printed output was produced on each of the image-receiving sheets, in a high-speed print mode, by use of a sublimation-type thermal transfer printer ASK2000 (trade name, manufactured by FUJIFILM Corporation). By use of signals to which neutral gray adjustment was made so that Sample 801 would give a visual density of 1.0 by the signals, gray solid images as printed output were produced in succession on 5 pieces of each sample sheet. Herein, the time interval between ejection of one printed piece and ejection of the next one was 8 seconds.

The evaluation of transferability in the vicinity of the maximum density, to which contributions of influences of the saturated adsorption amount of dyes and the thermal stability of a receptor polymer are relatively large, corresponds to the evaluation of total transfer performance of the receptor polymer, and the transferability at the visual density of 1.0 tends to have a relatively great contribution of a receptor polymer's influence on transferability.

#### (Image Evaluation)

##### (1) Evaluation of Developed-Color Density

The visual density of the gray image obtained under the above conditions was measured by Photographic Densitometer (trade name, manufactured by X-Rite Incorporated). In addition, surface quality of each of the gray solid images produced was observed, and the degree of evenness in solid image area and the condition of image failure occurrence were evaluated.

##### (2) Evaluation of Releasing Property (Adhesiveness)

The releasing property shown in releasing each image-receiving sheet from the ink sheet under the conditions of 35° C. and 80% RH, was evaluated by the frequency of sticking

occurrence determined as follows: 50 Sheets of prints with overall black images (black solid images) of maximum densities were output in succession, and the degrees of streaky unevenness (sticking) were evaluated by observation of their surfaces. Herein, the level at which transfer deviation occurred was regarded as problematic, and the ordinal number of a print on which the transfer deviation occurred first was defined as the frequency of sticking occurrence. At the same time, noises caused by this processing were caught and their volume was evaluated. These evaluation results were ranked as shown below, and the results are shown in Table 15. (Incidentally, the conditions mentioned above for evaluation are those apt to develop sticking.)

#### Evaluation Rank (Noises Caused by the Processing)

◎: Better results than the level for ○ were obtained.

○: Good results were obtained without any problems.

Δ: Results obtained showed tendencies to deteriorate, but they were still on a practically acceptable level.

X: Results obtained had problems, so they were on a practically unacceptable level.

Images were output to these Samples 801 to 809 and the resultant images were evaluated, in the same manner as in Example 1. In addition, gray solid images with the gray density of 0.6 were output, and the images produced on Samples 801 to 809 were observed. Results obtained are shown in Table 16.

TABLE 15

| Latex polymer | Vinyl chloride unit | Acrylic acid ester unit (Alcohol moiety) | Tg       |
|---------------|---------------------|------------------------------------------|----------|
| A             | 83                  | 17 (Methyl)                              | 69.5° C. |
| B             | 90                  | 10 (Ethyl)                               | 70.1° C. |
| C             | 93                  | 7 (Propyl)                               | 70.3° C. |
| D             | 95                  | 5 (Butyl)                                | 70.5° C. |
| E             | 96                  | 4 (2-Ethylhexyl)                         | 70° C.   |

TABLE 16

| Sample No. | Transfer density | The number of the sheet on which sticking occurred | Peel noise | Gray image                                                                                                                                     |
|------------|------------------|----------------------------------------------------|------------|------------------------------------------------------------------------------------------------------------------------------------------------|
| 801        | 1.00             | 5 pieces                                           | Δ          | The image produced was poor in a feeling of evenness, and developed fine unevenness in the density, but the sample was on an acceptable level. |
| 802        | 1.03             | 0 (none)                                           | ◎          | Excellent image quality free of image failures was attained.                                                                                   |
| 803        | 1.05             | 7 pieces                                           | ○          | Two spot failures were observed in the KG-size image area, but the sample was on an acceptable level.                                          |
| 804        | 1.12             | 3 pieces                                           | ○          | Three spot failures were observed in the KG-size image area, but the sample was on an acceptable level.                                        |
| 805        | 1.02             | 12 pieces                                          | Δ          | Not only two spot failures but also fine crack failures developed in the KG-size image area, but the sample was on an acceptable level.        |
| 806        | 1.05             | 1 piece                                            | ◎          | Not only two spot failures but also fine crack failures developed in the KG-size image area, but the sample was on an acceptable level.        |

TABLE 16-continued

| Sample No. | Transfer density        | The number of the sheet on which sticking occurred         | Peel noise | Gray image                                                                                                                               |
|------------|-------------------------|------------------------------------------------------------|------------|------------------------------------------------------------------------------------------------------------------------------------------|
| 807        | 0.73                    | 0 (none)                                                   | ○          | Density was seriously low, and no marketability was seen.                                                                                |
| 808        | 1.03                    | 12 pieces/<br>5 pieces<br>JAM                              | ○          | The gray image was poor in a feeling of evenness, and developed long-period of density unevenness. The sample was poor in marketability. |
| 809        | 1.12<br>2 pieces<br>JAM | The test piece was too sticky and did not pass the tester. | —          | Part of the image did not transfer upon peeling off the two sheets, and no marketability was seen.                                       |

(Note)

'KG-size image area' is an image area of size 4 inches x 6 inches

From the results shown in Table 16, it can be seen that Samples 801 to 806 meeting the requirements of the present invention ensured compatibility between transferability and ink-ribbon releasing property (sticking) and gave high-quality images, in comparison with Samples 807 to 809. Further, of the samples meeting the requirements of the present invention, it is found that Sample 802 using the latex polymer prepared by copolymerizing ethyl acrylate and vinyl chloride ensured high-quality images with specifically high compatibility between transferability and ink-ribbon adhesion, in comparison with other samples using other acrylate copolymers even having the same level of glass transition temperatures (Tg). In addition, it is found that Sample 804 using the latex polymer prepared by copolymerizing butyl acrylate and vinyl chloride was specifically excellent in transferability, as compared to other acrylate copolymers even having the same level of glass transition temperatures (Tg).

Having described our invention as related to the present embodiments, it is our intention that the invention not be limited by any of the details of the description, unless otherwise specified, but rather be construed broadly within its spirit and scope as set out in the accompanying claims.

What we claim is:

1. A heat-sensitive transfer image-receiving sheet, comprising;  
a support;  
at least one receptor layer containing a latex polymer and a water-soluble polymer, said latex polymer containing a repeating unit derived from vinyl chloride in a proportion of 50 mass % or above in the latex polymer; and  
at least one heat-insulation layer containing hollow latex polymeric particles and a water-soluble polymer, said at least one heat-insulation layer being provided between the support and the at least one receptor layer;  
wherein said hollow latex polymeric particles have an average particle diameter of 0.1 to 2  $\mu\text{m}$  and being non-foaming type hollow latex polymeric particles each having a capsule wall formed of a polystyrene, acrylic resin, or styrene/acrylic resin.
2. The heat-sensitive transfer image-receiving sheet according to claim 1, wherein the latex polymer contained in the at least one receptor layer is a copolymer of vinyl chloride and an acrylic acid ester.

3. The heat-sensitive transfer image-receiving sheet according to claim 2, wherein the latex polymer contained in the at least one receptor layer is a copolymer of vinyl chloride and at least two acrylic acid esters.

5 4. The heat-sensitive transfer image-receiving sheet according to claim 2, wherein the number of carbon atoms in an alcohol-derived moiety of the acrylic acid ester is 1 to 8.

5 10 5. The heat-sensitive transfer image-receiving sheet according to claim 2, wherein the number of carbon atoms in an alcohol-derived moiety of the acrylic acid ester is 1, and wherein a repeating unit derived from said acrylic acid ester is contained in the copolymer in a proportion of 10 to 45 mass %.

6 15 6. The heat-sensitive transfer image-receiving sheet according to claim 2, wherein the number of carbon atoms in an alcohol-derived moiety of the acrylic acid ester is 2, and wherein a repeating unit derived from said acrylic acid ester is contained in the copolymer in a proportion of 5 to 45 mass %.

7 20 7. The heat-sensitive transfer image-receiving sheet according to claim 2, wherein the number of carbon atoms in an alcohol-derived moiety of the acrylic acid ester is 3, and wherein a repeating unit derived from said acrylic acid ester is contained in the copolymer in a proportion of 5 to 35 mass %.

8 25 8. The heat-sensitive transfer image-receiving sheet according to claim 2, wherein the number of carbon atoms in an alcohol-derived moiety of the acrylic acid ester is 4, and wherein a repeating unit derived from said acrylic acid ester is contained in the copolymer in a proportion of 4 to 30 mass %.

9 30 9. The heat-sensitive transfer image-receiving sheet according to claim 2, wherein the number of carbon atoms in an alcohol-derived moiety of the acrylic acid ester is 6, and wherein a repeating unit derived from said acrylic acid ester is contained in the copolymer in a proportion of 3 to 28 mass %.

10 35 10. The heat-sensitive transfer image-receiving sheet according to claim 2, wherein the number of carbon atoms in an alcohol-derived moiety of each acrylic acid ester is 8, and wherein a repeating unit derived from said acrylic acid ester is contained in the copolymer in a proportion of 2 to 25 mass %.

11 40 11. The heat-sensitive transfer image-receiving sheet according to claim 1, wherein the latex polymer contained in the at least one receptor layer is a copolymer of vinyl chloride and vinyl acetate.

12 45 12. The heat-sensitive transfer image-receiving sheet according to claim 11, wherein a repeating unit derived from the vinyl acetate is contained in the copolymer in a proportion of 3 to 30 mass %.

13 50 13. The heat-sensitive transfer image-receiving sheet according to claim 1, wherein the latex polymer contained in the at least one receptor layer is a copolymer of vinyl chloride, at least one acrylic acid ester, and vinyl acetate.

14 55 14. The heat-sensitive transfer image-receiving sheet according to claim 1, which is produced through simultaneous coating of the at least one receptor layer and the at least one heat-insulating layer.

15 60 15. The heat-sensitive transfer image-receiving sheet according to claim 1, wherein the water-soluble polymer in the at least one heat-insulation layer is gelatin.

16 65 16. The heat-sensitive transfer image-receiving sheet according to claim 1, wherein the water-soluble polymer in the at least one receptor layer is gelatin.

17 70 17. The heat-sensitive transfer image-receiving sheet according to claim 1, wherein the at least one receptor layer or the at least one heat-insulation layer contains a hardener.